# EUROPEAN PATENT SPECIFICATION

(11) **EP 2 447 344 B1**
(45) Date of publication and mention of the grant of the patent: **24.07.2019**
(21) Application number: 10791159.6
(22) Date of filing: 25.06.2010
(51) Int. Cl.: C10L 1/183, C10L 10/00, C10L 1/222, C10L 1/223, C10L 1/224, C10L 1/228, C10L 1/232, C10L 1/233, C10L 1/238, C10L 1/2383, C10L 1/2387, C10L 1/24, C10L 10/18

(54) **DIESEL COMPOSITION AND PROCESS FOR IMPROVING OXIDATION STABILITY OF BIODIESEL**
DIESELZUSAMMENSETZUNG UND VERFAHREN ZUR VERBESSERUNG DER OXIDATIONSSTABILITÄT VON BIODIESEL
COMPOSITION DE DIESEL ET PROCÉDÉ POUR L'AMÉLIORATION DE LA STABILITÉ D'UN BIODIESEL À L'OXYDATION

(30) Priority: 26.06.2009 CN 200910087970; 30.07.2009 CN 200910089959; 19.08.2009 CN 200910090511; 19.08.2009 CN 200910090512
(43) Date of publication of application: 02.05.2012
(73) Proprietor: China Petroleum & Chemical Corporation, Beijing 100728 (CN); Research Institute Of Petroleum Processing, Sinopec, Beijing 100083 (CN)
(72) Inventor: LIN, Jianmin, Beijing 100083 (CN); ZHANG, Yongguang, Beijing 100083 (CN); ZHANG, Jianrong, Beijing 100083 (CN); LI, Hang, Beijing 100083 (CN); LI, Shuai, Beijing 100083 (CN)
(74) Representative: Lang, Johannes
(86) International application number: PCT/CN2010/000950
(87) International publication number: WO 2010/148652

(56) References cited:
- EP-A1- 1 568 757
- EP-A2- 1 847 583
- EP-A2- 1 847 584
- WO-A1-2007/145738
- WO-A1-2009/029373
- WO-A2-2008/049822
- WO-A2-2008/124390
- CN-A- 101 319 155
- US-A- 6 083 288
- US-A1- 2009 139 135

## Description

### Technical Field

The present invention relates to a diesel composition and a method of increasing the oxidation stability of biodiesel.

### Background Art

With the accelerated dieselization of vehicles all over the world, the demand for diesel will be larger and larger, furthurmore, as petroleum resources are drying up day by day and people are more and more conscious of environmental issues, countries worldwide are greatly promoted to expedite the development of alternative fuels for diesel engine. Therefore, biodiesel, which is very environmentally-friendly and renewable, attracts much attention all over the world.

Biodiesel (BD100), also called fatty acid methyl ester, is obtained by transesterrification of oils from oil crops, such as soybeans and rapeseeds, the fruits of oil plants, such as *Elaeis* and *Pistacia chinesis Bunge,* and oil water plants, such as algae as well as animal fats, used cooking oils thrown away by restaurants or families, and the like with alcohols (methanol, ethanol), and is a clean biofuel. Biodiesel has three advantages of being renewable, clean and safe, and is strategically significant to the agricultural structure adjustment, energy safety and protection of the ecological environment. At present, China is a net importer of petroleum and has limited petroleum reserves, and importing petroleum in huge quantity threatens the energy safety in China; thus, the study on and production of biodiesel is practically significant in China.

However, because of the starting materials and processing steps, some biodiesels have very poor oxidation stability, causing great difficulties in their use and storage. Biodiesels having poor oxidation stability tends to produce the following aging products: 1) insoluble polymers (gelatines and fatlute), which will cause clogging of engine filters and coking of jet pumps, and result in an increased smoke discharge and difficulty in start-up; 2) soluble polymers, which can form resin-like materials in engines, and may possibly result in flameout and difficulty in start-up; 3) aging acids, which will erode metal parts in engines; 4) peroxides, which will cause aging and embrittlement of rubber parts, resulting in fuel leak.

The European biodiesel standard EN 14214:2003, the Australian biodiesel standard (Draft 2003), the New Zealand biodiesel standard NZS 7500:2005, the Brazilian biodiesel standard ANP255 (2003), the Indian biodiesel standard IS 15607:2005, the South African biodiesel standard SANS 1935:2004 and the Chinese national standard GB/T 20828-2007 for the biodiesel (BD100) for blended fuel diesel engines all prescribe that the oxidation stability of biodiesel is shown by an induction period of not shorter than 6 hours at 110 °C, as measured by the EN 14112:2003 method.

As generally known, olefins, diolefins and non-hydrocarbons, such as sulphides and nitrides, in petroleum diesel (usually known as diesel, petroleum diesel being introduced here is to be distinguished from biodiesel) produce a series of oxidation intermediate products in the presence of oxygen, and generate insoluble precipitates by condensation. Such insoluble particles generated during the storage of petroleum diesel will influence the properties of the fuel, resulting in the clogging of filter systems, and causing the parts of fuel systems to malfunction, such that the atomization of the oil sprayed will be affected, leading to incomplete combustion, and even the formation of excess carbon deposit in engines to clog spray nozzles. Since the oxidation stability of biodiesel is inferior to that of petroleum diesel, the above problems will be worse if biodiesel is blended with petroleum diesel. The most obvious manifestation is that the stability of a biodiesel-containing blended fuel is inferior to that of petroleum diesel.

The above problems can be solved or mitigated by the addition of additives. One way is to add antioxidants in pure biodiesel to delay its oxidation, hence mitigating the harms made by the aging products; the other way is to add stabilizers in petroleum diesel or a biodiesel-containing blended fuel to improve the stability of the blended fuel. A stabilizer is capable of terminating, weakening or interfering with various oxidation reactions to inhibit oil deterioration and then improve the stability.

CN 1742072A discloses a process for increasing the storage stability of biodiesel, comprising adding a stock solution comprising 15-60 wt.% 2,4-di-tert-butylhydroxy toluene dissolved in biodiesel, into the biodiesel to be stabilized until the 2,4-di-tert-butylhydroxy toluene reaches a concentration of 0.005-2 wt.% with respect to the total solution of biodiesel.

CN 1847368A discloses a method of increasing the oxidation stability of biodiesel, comprising adding a bisphenol-type antioxidant, such as 4,4'-methylenebis[2,6-di-tert-butylphenol] or 2,2'-methylenebis[6-tert-butyl-4-methylphenol], to the biodiesel to be stabilized in a quantity of 10-20000 ppm (w/w).

CN 1847369A discloses a method of increasing the oxidation stability of biodiesel, comprising adding a primary antioxidant having a melting point of less than or equal to 40 °C to the biodiesel to be stabilized in an amount of from 10 to 20000 ppm (w/w), where the primary antioxidant comprises alkylphenol.

US2007/113467A1 discloses a fuel composition having an improved oxidation stability, which comprises biodiesel and at least one antioxidant selected from the group consisting of propyl gallate, 1,2,3-trihydroxybenzene, 2,6-di-tert-butyl-p-methylphenol, butylated hydroxyanisole, dilauryl thiodipropinate, tocopherol, and quinoline derivatives.

CN 101144040A and CN 101353601A disclose methods of improving the oxidation stability of biodiesel by using an arylamine-type antioxidant.

The above methods of increasing the oxidation stability of biodiesel by using conventional antioxidants are effective in some degree, but require a relatively large amount of antioxidants, and in the meantime do not have a satisfactory effect of improving the stability of a biodiesel-containing blended fuel.

US 2009/0139135 A1 discloses a method for improving the stability of biodiesel comprising adding an alkyl phenol amine aldehyde condensate additive to the biodiesel. WO 2008/124390 A2 refers to a fuel composition comprising a specific fatty acid ester, a nitrogen containing detergent and a phenolic antioxidant. EP 1 847 583 A2 and EP 1 847 584 A2 relate to the prevention or retardation of the oxidation of oils derived from plant or animal materials.

### Contents of the Invention

One of the object of the present invention is to provide a diesel composition with an improved oxidation stability of biodiesel or a superior stability and a method of improving the oxidation stability of biodiesel in order to remove the above-mentioned disadvantages of the prior art of requiring a large amount of antioxidant and having a poor effect of improving the stability of a biodiesel-containing blended fuel.

The present invention provides according to claim 1 a diesel composition comprising a base diesel and an additive composition. Said base diesel comprises biodiesel, and said additive composition comprises component (a) and component (b), wherein said component (a) is an arylamine-type antioxidant which is a substituted p-phenylene diamine, and said component (b) is one or more polyamines or derivatives thereof.

The present invention further provides a method of increasing the oxidation stability of biodiesel, comprising adding, in a biodiesel-containing base diesel, an additive, wherein said additive is the additive composition provided by the present invention.

The diesel composition of the present invention has a superior oxidation stability, and component (a) and component (b) surprisingly show synergism, i.e., a much better antioxidative effect than a single antioxidant. Component (b) can be regarded as a co-antioxidant, which surprisingly greatly enhances the effect of the antioxidant. Thus, in reaching the same oxidation stability, the amount of component (a) in the biodiesel composition can be reduced considerably, and in particular when component (a) is expensive or is toxic or corrosive in some degree. It is of great significance to reduce the amount of component (a). Especially, when it simultaneously comprises component (a), component (b) and component (c), the diesel composition of the present invention has a remarkably improved antioxidative property due to the significant synergism of the components.

### Specific Embodiments

In the diesel composition according to the present invention, the amount of additive can be selected from a relatively wide range, such as 50-10000 ppm, preferably 80-8000 ppm, and more preferably 100-5000 ppm, on the basis of the amount of the base diesel.

The weight ratio of said component (b) to said component (a) is 0.01-100: 1, preferably 0.02-50: 1, more preferably 0.05-10: 1, even more preferably 0.2-5:1.

### Component (a)

Component (a) is at least one arylamine-type antioxidant which is a substituted p-phenylene diamine.

Said substituted p-phenylene diamine-type antioxidant can be a product obtained by substitution of the hydrogen atom(s) of the amino group(s) (-NH₂) in the p-phenylene diamine with one or more of alkyl, aryl, aralkyl, alkylaryl, hydrocarbylacyl, hydrocarbylsulfonyl and hydrocarbylacyloxy. When two hydrogen atoms of the amino groups are substituted, they may be hydrogen on the same amino group or on two different amino groups. Moreover, when there are more than two substituents, the substituents may be the same or different. In other words, said substituted p-phenylene diamine-type antioxidant can be one or more of mono-alkyl substituted p-phenylene diamine, mono-aryl substituted p-phenylene diamine, mono-alkylaryl substituted p-phenylene diamine, mono-arylalkyl substituted p-phenylene diamine, mono-hydrocarbylacyl substituted p-phenylene diamine, mono-hydrocarbylsulfonyl substituted p-phenylene diamine, mono-hydrocarbylacyloxy substituted p-phenylene diamine, N-alkyl-N'-alkyl substituted p-phenylene diamine, N-aryl-N'-alkyl substituted p-phenylene diamine, N-alkyl-N'-alkylaryl substituted p-phenylene diamine, N-aryl-N'-alkyl substituted p-phenylene diamine, N-arylalkyl-N'-alkyl substituted p-phenylene diamine, N-arylalkyl-N'-aryl substituted p-phenylene diamine, N-arylalkyl-N'-hydrocarbylacyl substituted p-phenylene diamine, N-arylalkyl-N'-hydrocarbylsulfonyl substituted p-phenylene diamine, N-arylalkyl-N'-hydrocarbylacyloxy substituted p-phenylene diamine, N-aryl-N'-hydrocarbylacyl substituted p-phenylene diamine, N-alkyl-N'-hydrocarbylsulfonyl substituted p-phenylene diamine, N-alkyl-N'-hydrocarbylacyloxy substituted p-phenylene diamine, N-aryl-N'-hydrocarbylacyl substituted p-phenylene diamine, N-alkyl-N'-hydrocarbylsulfonyl substituted p-phenylene diamine, N-alkyl-N'-hydrocarbylacyloxy substituted p-phenylene diamine, N-alkylaryl-N'-hydrocarbylacyl substituted p-phenylene diamine, N-alkylaryl-N'-hydrocarbylsulfonyl substituted p-phenylene diamine, N-alkylaryl-N'-hydrocarbylacyloxy substituted p-phenylene diamine, N,N-bis-alkyl substituted p-phenylene diamine, N,N-bis-aryl substituted p-phenylene diamine, N,N-bis-alkylaryl substituted p-phenylene diamine, N,N-bis-arylalkyl substituted p-phenylene diamine, N,N-bis-hydrocarbylsulfonyl substituted p-phenylene diamine, N,N-bis-hydrocarbylacyl substituted p-phenylene diamine, and N,N-bis-hydrocarbylacyloxy substituted p-phenylene diamine. Each substituent preferably has 1 to 20 carbon atoms, and in terms of an alkyl radical, it preferably has 4 to 10 carbon atoms.

Specifically, said substituted p-phenylene diamine-type antioxidant includes, but is not limited to, one or more of the following:
N-phenyl-N'-cyclohexyl-p-phenylene diamine (antioxidant 4010);
N,N-(1,3-dimethylbutyl)-N'-phenyl-p-phenylene diamine (antioxidant 4020);
N,N'-bis-(1,4-dimethylamyl) p-phenylene diamine (antioxidant 4030);
N-p-tolyl-N'-(1,3-dimethylbutyl) p-phenylene diamine (antioxidant 4040);
N,N'-diheptyl-p-phenylene diamine (antioxidant 788);
N-isopropyl-N'-phenyl-p-phenylene diamine (antioxidant 4010NA);
N-isopropyl-N'-p-tolyl-p-phenylene diamine (antioxidant methyl4010NA);
N,N'-xylyl-p-phenylene diamine (antioxidant PPD-A);
N,N'-diphenyl-p-phenylene diamine (antioxidant H);
N,N'-di-(β-naphthyl) p-phenylene diamine (antioxidant DNP);
N,N'-di-sec-butyl-p-phenylene diamine (antioxidant U-5);
N,N'-dioctyl-p-phenylene diamine (antioxidant 88);
N,N'-bis-(1-methylheptyl) p-phenylene diamine (antioxidant 288);
N,N'-bis-(1-ethyl-3-methylamyl) p-phenylene diamine (antioxidant 8L);
N,N'-bis-(1,4-dimethylbutyl) p-phenylene diamine (antioxidant 66);
N-octyl-N'-phenyl-p-phenylene diamine (antioxidant 688);
N-isobutyl-N'-phenyl-p-phenylene diamine (antioxidant 5L);
N,N'-dimethyl-N,N'-bis-(1-methylpropyl) p-phenylene diamine (antioxidant 32);
N-(p-toluene sulfonyl)-N'-phenyl-p-phenylene diamine (antioxidant TPPD);
N-(3-methylpropenylacryloxo-2-hydroxypropyl)-N'-phenyl-p-phenylene diamine (antioxidant G-1);
N-(3-anilinophenyl)methylacrylamide;
N-hexyl-N'-phenyl-p-phenylene diamine.

In the present invention, the substituted p-phenylene diamine-type antioxidant is preferably one or more dialkyl p-phenylene diamines wherein the hydrogen atoms of the amino groups therein are substituted by two alkyl radicals, two aryl radicals or one alkyl radical and one aryl radical, and particularly preferably one or more substituted dialkyl p-phenylene diamines, wherein the two amino groups therein are independently substituted with an alkyl radical having 4 to 10 carbon atoms or an aryl radical having 6 to 15 carbon atoms, such as, one or more of N,N'-diheptyl-p-phenylene diamine, N,N'-di-sec-butyl-p-phenylene diamine, N,N'-bis-(1-ethyl-3-methylamyl)p-phenylene diamine, N,N'-bis-(1,4-dimethylbutyl) p-phenylene diamine, N,N'-dioctyl-p-phenylene diamine, and N,N'-bis-(1-methylheptyl)p-phenylene diamine.

In the present invention, the component (a) is most preferably one or more of N,N-(1,3-dimethylbutyl)-N'-phenyl-p-phenylene diamine, N-octyl-N'-phenyl-p-phenylene diamine, N,N'-diheptyl-p-phenylene diamine, N,N'-di-sec-butyl-p-phenylene diamine, N,N'-dioctyl-p-phenylene diamine, N,N'-bis-(1-methylheptyl)p-phenylene diamine, N,N'-bis-(1-ethyl-3-methylamyl) p-phenylene diamine and N,N'-bis-(1,4-dimethylbutyl) p-phenylene diamine.

### Component (b)

A polyamine is an organic amine having the structure shown by the structural formula (A):
wherein R₁ and R₂ are each independently H, a hydrocarbyl having from 1 to 30 carbon atoms or a hydrocarbyl having from 1 to 30 carbon atoms and bearing a group selected from carbonyl, hydroxyl, carboxyl, ester group, acyl, alkoxy, nitro, cyano, halo, amine group or amino, wherein said hydrocarbyl having from 1 to 30 carbon atoms and a group selected from carbonyl, hydroxyl, carboxyl, ester group, acyl, alkoxy, nitro, cyano, halo, amine group or amino can be further substituted by a hydrocarbyl having from 1 to 30 carbon atoms or a group selected from carbonyl, hydroxyl, carboxyl, ester group, acyl, alkoxy, nitro, cyano, halo, amine group or amino, or can form a ring,
with the proviso that said organic amine comprises two or more N atoms.

The polyamine of component (b) is one or more of the following amines:
a polyether diamine of formula (A1):
wherein x1 is an integer from 1 to 10, R₄ is H or a hydrocarbyl having 1 to 30 carbon atoms, and R₅ is H or methyl. Preferably, said polyether diamine is a polyether diamine with the CAS number 9046-10-0, having a number average molecular weight of 400;
a polyene polyamine of the structural formula:

   H₂N[(CH₂)ₓ₂NH]_{y1}R₆
wherein x2 is an integer from 2 to 4, y1 is an integer from 1 to 8, and R₆ is H or a hydrocarbyl having 1 to 30 carbon atoms, and/or a condensate of said polyene polyamine with ethylene oxide and/or propylene oxide, such as one or more of ethylene diamine, diethylene triamine, triethylene tetramine, tetraethylene pentamine, pentaethylene hexamine, hexaethylene heptamine, heptaethylene octamine, propylene diamine, dipropylene triamine, tripropylene tetramine, tetrapropylene pentamine, pentapropylene hexamine, hexapropylene heptamine, heptapropylene octamine, and N,N'-bis-(3-aminopropyl)-ethylene diamine, or one or more polyene polyamines wherein R₆ is n-butyl, n-amyl, n-hexyl, n-heptyl, n-octyl, n-nonyl, n-decyl, n-undecyl, n-dodecyl, n-tetradecyl, n-hexadecyl, n-octadecyl, n-eicosyl, n-didodecyl; isobutyl, tert-butyl, iso-amyl, neo-amyl, iso-hexyl, iso-heptyl, iso-octyl, iso-nonyl, iso-decyl, iso-dodecyl, iso-tetradecyl, iso-hexadecyl, iso-octadecyl, iso-eicosyl, 9-octadecene, phenylmethyl, phenylethyl or phenylpropyl;
an imidazoline-type polyamine of the formula (A2):
wherein y2 is an integer from 0 to 5, and R₇ is a hydrocarbyl having 1 to 24 carbon atoms, and preferably, y2 is an integer from 1 to 3, and R₇ is C₆-C₂₀ alkyl or alkenyl;
a piperazine-type polyamine being N-(2-aminoethyl) piperazine or N,N'-di-(aminoethyl) piperazine;
a piperidine-type polyamine, which is preferably 4-amino-2,2,6,6-tetramethylpiperidine or 1-(2-aminoethyl) piperidine;
a tertiary amine containing polyamine of the formula (A4), (A5) or (A6):
wherein R₉ and R₁₀ are hydrocarbyls having 1 to 24 carbon atoms, and x4 is an integer from 0 to 10, such as one or more of N,N-dimethyl-1,3-propylene diamine, N,N-diethyl-1,3-propylene diamine, N,N-dibutyl-1,3-propylene diamine, N,N-dimethyl-1,4-butane diamine, N,N-diethyl-1,4-butane diamine, and N,N-dimethyl-1,6-hexanediamine;
wherein x5 is an integer from 1 to 10, said polyamine being preferably tri-(2-aminoetyl) amine;
wherein R₁₁ is a hydrocarbyl having 1 to 24 carbon atoms, and x6 is an integer from 1 to 10, and preferably an integer from 2 to 6, said polyamine being preferably N,N-bis-(3-aminopropyl) methylamine.

The term "hydrocarbyl" herein refers to hydrocarbon substituents, including aliphatic, alicyclic, aryl and heterocyclic substituents.

The aliphatic hydrocarbyl may be a saturated hydrocarbyl or unsaturated hydrocarbyl having a double or triple bond, including alkyl, alkenyl, and alkynyl.

Unless otherwise stated, the term "alkyl" in the present invention refers to linear or branched alkyl typically having 1 to 30, preferably 1 to 18 carbon atoms, such as methyl, ethyl, n-propyl, isopropyl, n-butyl, isobutyl, sec-butyl, tert-butyl, n-amyl, iso-amyl, 2-methylbutyl, neo-amyl, 3-amyl, n-hexyl, 4-methylamyl, 3-methylamyl, 2-methylamyl, 1-methylamyl, 3,3-dimethylbutyl, 2,2-dimethylbutyl, 1,1-dimethylbutyl, 1,2-dimethylbutyl, 1,3-dimethylbutyl, 2,3-dimethylbutyl, 2-ethylbutyl, 1-methyl-2-methylpropyl, n-heptyl, n-octyl, n-nonyl, n-decyl, n-undecyl, n-dodecyl, n-tridecyl, n-tetradecyl, n-pentadecyl, n-hexadecyl, n-heptadecyl, n-octadecyl and the like.

Unless otherwise stated, the term "alkenyl" in the present invention refers to linear or branched alkenyl having a double bond and typically having 2 to 30, preferably 2 to 6 carbon atoms, such as vinyl, 1-propenyl, 1-propyl-2-ene, 2-propenyl, 1-butenyl, 1-butyl-2-ene, 1-butyl-3-ene, 1-methyl-1-propenyl, 2-methyl-1-propenyl, 1-methyl-1-propyl-2-ene, 2-methyl-1-propyl-2-ene, 1-pentenyl, 1-amyl-2-ene, 1-amyl-3-ene, 1-amyl-4-ene, 1-methyl-1-butenyl, 2-methyl-1-butenyl, 3-methyl-1-butenyl, 1-methyl-1-butyl-2-ene, 2-methyl-1-butyl-2-ene, 3-methyl-1-butyl-2-ene, 1-methyl-1-butyl-3-ene, 2-methyl-1-butyl-3-ene, 3-methyl-1-butyl-3-ene, 1-hexenyl, 1-hexyl-2-ene, 1-hexyl-3-ene, 1-hexyl-4-ene, 1-hexyl-5-ene, 1-methyl-1-pentenyl, 2-methyl-1-pentenyl, 3-methyl-1-pentenyl, 4-methyl-1-pentenyl, 1 -methyl-1 -amyl-2-ene, 2-methyl-1-amyl-2-ene, 3-methyl-1-amyl-2-ene, 4-methyl-1-amyl-2-ene, 1 -methyl- 1 -amyl-3-ene, 2-methyl-1-amyl-3-ene, 3-methyl-1-amyl-3-ene, 4-methyl-1-amyl-3-ene, 1-methyl-1-amyl-4-ene, 2-methyl-1-amyl-4-ene, 3-methyl-1-amyl-4-ene, 4-methyl-1-amyl-4-ene, and the like.

Unless otherwise stated, the term "alkynyl" in the present invention refers to linear or branched alkynyl having a triple bond and typically having 2 to 30, preferably 2 to 6 carbon atoms, such as ethynyl, 1-propynyl, 1-propyl-2-yne, 1-butynyl, 1-butyl-2-yne, 1-butyl-3-yne, 1-pentynyl, 1-amyl-2-yne, 1-amyl-3-yne, 1-amyl-4-yne, 3-methyl-1-butynyl, 1-methyl-1-butyl-2-yne, 1-methyl-1-butyl-3-yne, 2-methyl-1-butyl-3-yne, 1-hexynyl, 1-hexyl-2-yne, 1-hexyl-3-yne, 1-hexyl-4-yne, 1-hexyl-5-yne, 3-methyl-1-pentynyl, 4-methyl-1-pentynyl, 1 -methyl-1 -amyl-2-yne, 4-methyl-1-amyl-2-yne, 1-methyl-1-amyl-3-yne, 2-methyl-1-amyl-3-yne, and the like.

Unless otherwise stated, the term "alicyclic hydrocarbyl" in the present invention refers to saturated cyclohydrocarbyl or unsaturated cyclohydrocarbyl having a double or a triple bond, including cycloalkyl and cycloalkenyl.

Unless otherwise stated, the "cycloalkyl" is selected from the group consisting of cyclopropyl, cyclobutyl, cyclopentyl, cyclohexyl, cycloheptyl, cyclooctyl, and the like. Cyclopropyl, cyclopentyl, cyclohexyl etc. are prefered, and cyclopropyl and cyclohexyl are more preferred.

Unless otherwise stated, the "cycloalkenyl" is selected from the group consisting of cyclobutenyl, cyclopentenyl, cyclohexenyl, cyclopentadienyl, cyclohexadienyl, cycloheptadienyl, cyclooctadienyl, and the like, of which cyclopentenyl, cyclohexenyl, cyclopentadienyl, cyclohexadienyl etc. are preferred, and cyclopentenyl and cyclopentadienyl are more preferred.

Unless otherwise stated, the term "aryl" in the present invention refers to any functional groups or substituents derived from simple aromatic rings, such as phenyl, and substituted phenyl (e.g., benzyl, phenylethyl, methoxyphenyl, dinitrophenyl, tert-butoxycarbonylphenyl, and the like), and fused aromatic rings, such as, naphthyl, anthryl, phenanthrenyl, and substituted naphthyl, and the like.

Unless otherwise stated, the term "heterocyclic substituent" in the present invention comprises a 3-8 membered, saturated cyclic structure containing heteroatoms, or a 3-8 membered, unsaturated cyclic structure containing heteroatoms.

Said "3-8 membered, saturated cyclic structure containing heteroatoms" refers to a 3-8 membered cyclic structure having no unsaturated bonds in the ring, such as, azacyclopropane (aziridine), 2H-azacyclopropane, diazacyclopropane, azacyclobutane, 1,2-diazacyclobutane, pyrrolidine, imidazolidine, pyrazolidine, hydrogenated pyridone, piperidine , piperazine, ethylene oxide, dioxacyclopropane, thiacyclopropane, oxacyclobutane, 1,2-dioxacyclobutane, thiacyclobutane, tetrahydrofuran, tetrahydrothiophene, 1,3-dioxacyclopentane, 1,3-dithiacyclopentane, tetrahydropyran, 1,4-dioxacyclohexane, 1,3-dioxacyclohexane, 1,3-oxythiacyclohexane, oxyazacyclopropane, oxazole, morpholine and the like.

Said "3-8 membered, unsaturated cyclic structure containing heteroatoms" refers to a 3-8 membered cyclic structure having unsaturated bonds, such as 3H-diazacyclopropene, azacyclobutadiene, 1,2-diazacyclobutene, pyrrole, dihydropyrrole, imidazole, 4,5-dihydroimidazole, pyrazole, 4,5-dihydropyrazole, 1,2,3-triazole, 1,2,4-triazole, tetrazole, pyridine, 2-pyridone, 4-pyridone, pyridazine, pyrimidine, pyrazine, 1,2,3-triazine, 1,2,4-triazine, 1,3,5-triazine, 1,2,4,5-tetrazine, azacycloheptantriene, 1,2-diazacycloheptantriene, 1,3-diazacycloheptantriene, 1,4-diazacycloheptantriene, azacyclooctatetraene, 1,4-dihydro-1,4-diazacyclooctatriene,1,2-dithiacyclobutene, furan, thiophene, 2,5-dihydrothiophene, 1,2-dithiacyclopentene, 2H-pyran, 2H-pyran-2-one, 3,4-dihydro-2H-pyran, 4H-pyran, 4H-pyran-4-one, 1,4-dioxacyclohexadiene, 1,4-dithiacyclohexadiene, 1,4-oxathiacyclohexadiene, oxacycloheptantriene, thiacycloheptantriene, 1,4-dioxacyclooctatriene, oxazole, 4,5-dihydrooxazole, iso-oxazole, 4,5-dihydroiso-oxazole, 2,3-dihydroiso-oxazole, 1,2,3-oxdiazole, 1,2,5-oxdiazole, thiazole, 4,5-dihydrothiazole, iso-thiazole, 1,2,3-thiadiazole, 1,2,4-thiadiazole, 1,3,4-thiadiazole, 2H-1,2-oxazine, 4H-1,2-oxazine, 6H-1,2-oxazine, 2H-1,3-oxazine, 4H-1,3-oxazine, 5,6-dihydro-4H-1,3-oxazine, 6H-1,3-oxazine, 2H-1,4-oxazine, 4H-1,4-oxazine, 2H-1,3-thiazine, 4H-1,3-thiazine, 5,6-dihydro-4H-1,3-thiazine, 6H-1,3-thiazine, 2H-1,4-thiazine, 4H-1,4-thiazine, morpholine, and the like Pyrrole, dihydropyrrole, imidazole, 4,5-dihydroimidazole, pyrazole, 4,5-dihydropyrazole, pyridine, pyridazine, pyrimidine, pyrazine, furan, thiophene, 2,5-dihydrothiophene, 2H-pyran, 2H-pyran-2-one, 3,4-dihydro-2H-pyran, 4H-pyran, 4H-pyran-4-one, 1,4-dioxacyclohexadiene, 1,4-dithiacyclohexadiene, 1,4-oxathiacyclohexadiene, oxazole, 4,5-dihydrooxazole, iso-oxazole, 4,5-dihydroiso-oxazole, 2,3-dihydroiso-oxazole, 1,2,3-oxdiazole, 1,2,5-oxdiazole, thiazole, 4,5-dihydrothiazole, iso-thiazole, 1,2,3-thiadiazole, 1,2,4-thiadiazole, 1,3,4-thiadiazole etc. are preferred.

The above-mentioned hydrocarbyl having 1 to 30 carbon atoms may further carry a group selected from the group consisting of carbonyl, hydroxy (-OH), carboxyl (-COOH), ester groups, acyl, alkoxy, nitro, cyano, halo and amino.

The term "halo" in the present invention refers to fluoro, chloro, bromo, iodo and the like, of which fluoro, chloro and bromo are preferred, and chloro is more preferred.

The "alkoxy" in the present invention has a linear or branched alkyl and 1 to 30, preferably 1 to 18, carbon atoms, such as, methoxy, ethoxy, n-propoxy, iso-propoxy, n-butoxy, iso-butoxy, sec-butoxy, tert-butoxy, n-pentoxy, iso-pentoxy, 2-methylbutoxy, neo-pentoxy, 3-pentoxy, n-hexoxy, 4-methylpentoxy, 3-methylpentoxy, 2-methylpentoxy, 1-methylpentoxy, 3,3-dimethylbutoxy, 2,2-dimethylbutoxy, 1,1-dimethylbutoxy, 1,2-dimethylbutoxy, 1,3-dimethylbutoxy, 2,3-dimethylbutoxy, 2-ethylbutoxy, 1-methyl-2-methylpropoxy, n-heptoxy, n-octoxy, n-nonyloxy, n-decyloxy, n-undecyloxy, n-dodecyloxy, n-tridecyloxy, n-tetradecyloxy, n-pentadecyloxy, n-hexadecyloxy, n-heptadecyloxy, n-octadecyloxy and the like.

The "ester group" in the present invention has a linear or branched alkyl and 1 to 30, preferably 1 to 18, carbon atoms, such as, methyl ester group, ethyl ester group, n-propyl ester group, iso- propyl ester group, n-butyl ester group, iso-butyl ester group, sec-butyl ester group, tert-butyl ester group, n-pentyl ester group, iso-pentyl ester group, 2-methylbutyl ester group, neo-pentyl ester group, 3- pentyl ester group, n-hexyl ester group, 4-methylpentyl ester group, 3-methylpentyl ester group, 2-methylpentyl ester group, 1-methylpentyl ester group, n-heptyl ester group, n-octyl ester group, n-nonyl ester group, n-decyl ester group, n-undecyl ester group, n-dodecyl ester group, n-tridecyl ester group, n-tetradecyl ester group, n-pentadecyl ester group, n-hexadecyl ester group, n-heptadecyl ester group, n-octadecyl ester group or the like.

The "acyl" in the present invention has a linear or branched alkyl and 1 to 30, preferably 1 to 18, carbon atoms, such as, formyl, acetyl, n-propionyl, iso-propionyl, n-butyryl, iso-butyryl, sec-butyryl, tert-butyryl, n-valeryl, iso-valeryl, 2-methylbutyryl, neo-valeryl, 3-valeryl, n-hexanoyl, 4-methylvaleryl, 3-methylvaleryl, 2-methylvaleryl, 1-methylvaleryl, n-heptanoyl, n-octanoyl, n-nonanoyl, n-decanoyl, n-undecanoyl, n-dodecanoyl, n-tridecanoyl, n-tetradecanoyl, n-pentadecanoyl, n-hexadecanoyl, n-heptadecanoyl, n-octadecanoyl and the like.

Unless otherwise stated, the "hydrocarbylene" in the present invention is formed by removal of one hydrogen atom from the "hydrocarbyl" defined above. Said hydrocarbylene has 1 to 30, preferably 1 to 24 carbon atoms.

Said derivatives of polyamines are the reaction products of the ammonolysis reaction of one or more organic acids having 6 to 40 carbon atoms, acyl halides having 6 to 40 carbon atoms, or organic acid alkyl esters having 6 to 40 carbon atoms with the above-mentioned polyamines. Further preferred are the reaction products of the ammonolysis reaction of one or more monofatty acids having 6 to 40 carbon atoms, fatty acyl halides having 6 to 40 carbon atoms, or fatty acid alkyl esters having 6 to 40 carbon atoms with the above-mentioned polyamines. Said ammonolysis reaction refers to a metathetic reaction of one or more of fatty acids, fatty acyl halides and fatty acid alkyl esters with ammonia and/or amine to produce an amide. The reaction product of the above reaction can be used directly as component (b) without being isolated and purified, or the amidate alone therein can be used as component (b) after isolation and purification. Without isolation and purification, the mixture primarily comprises an amidate, and typically further comprises some unreacted starting materials and other reaction products, such as ammonium salts or alcohols. The specific composition of the mixture varies slightly depending on the reaction conditions.

The amidate according to the present invention is commercially available or obtained through a variety of known amidation reactions. For example, it is obtained by the ammonolysis reaction of an acid of formula (B1) or an ester of formula (B2) with a polyamine of formula (A) in a molar ratio of 1: (0.5-2). In said ammonolysis reaction, said polyamine is present in a stoichiometric amount or a slightly excess amount relative to said acid, acyl halide or ester. For example, an organic monocarboxylic acid of formula (B1) or an organic monocarboxylate of formula (B2) reacts with a polyamine of formula (A) in a molar ratio of 1: (1-2), and the product obtained from the ammonolysis reaction is preferably used directly as component (b) of the present invention without being isolated and purified. wherein R is a hydrocarbyl having 6 to 40, preferably 8 to 36 carbon atoms.

In formula (B1), R is a hydrocarbyl having 6 to 40, preferably 8 to 36 carbon atoms. The term "hydrocarbyl" used herein is as defined above, and refers to hydrocarbon substituents, including aliphatic, alicyclic, aryl and heterocyclic substituents. The aliphatic hydrocarbyl may be a saturated hydrocarbyl or unsaturated hydrocarbyl having a double or triple bond. For example, formula (B1) may be a fatty acid, a naphthenic acid, an aromatic acid, or a substituted aromatic acid, and preferably a fatty acid, which may be a monoacid, or a polyacid, such as a diacid. Said acid can be an acid alone or a mixture of acids, such as one or more fatty acids of vegetable oils, e.g., palmitic acid, soybean oil acid, peanut oil acid, rapeseed oil acid, ricinoleic acid, and tall oil fatty acid, and is most preferably one or more liquid acids at normal temperature, e.g. oleic acid, linoleic acid, linolenic acid, dimer oleic acid, dimer linoleic acid, industrial dimer acids, soybean oil acid, peanut oil acid, rapeseed oil acid, ricinoleic acid, and tall oil fatty acid. The substituted aromatic acids are, for example, substituted benzoic acid and/or alkyl substituted salicylic acid, and the like. The fatty acids according to the present invention are C6-C40 fatty acids, preferably one or more of caproic acid, adipic acid, octanoic acid, isooctanoic acid (2-ethylcaproic acid), capric acid, dodecanic acid (lauric acid), tetradecanoic acid, hexadecanoic acid (palmitic acid), octadecanoic acid (stearic acid), oleic acid, linoleic acid, linolenic acid, ricinolic acid, eicosenoic acid, arachidic acid, erucic acid, docosenoic acid, dimers of oleic acid and/or linoleic acid, dimer oleic acid, dimer linoleic acid, industrial dimer acids, soybean oil acid, peanut oil acid, rapeseed oil acid, ricinoleic acid, and tall oil fatty acid.

In formula (B2), R' is an alkyl having 1 to 5 carbon atoms, preferably methyl, ethyl, propyl, or isopropyl. Formula (B2) is an ester of the acid of formula (B1), preferably a methyl ester of the acid of formula (B1) or a mixture thereof, and particularly preferably a biodiesel.

Component (b) preferably comprises one or more of the following amidates, wherein the carbonyl moiety of the amide has 6 to 40, preferably 8 to 36, carbon atoms:
NH₂[(CH₂)ₓ₂NH]_{y1}COC₇H₁₅ (octanoic acid or isooctanoic acid amide),
NH₂[(CH₂)ₓ₂NH]_{y1}COC₈H₁₇ (nonanoic acid amide),
NH₂[(CH₂)ₓ₂NH]_{y1}COC₉H₁₉ (capric acid amide),
NH₂[(CH₂)ₓ₂NH]_{y1}COC₁₁H₂₃ (lauric acid amide),
NH₂[(CH₂)ₓ₂NH]_{y1}COC₁₃H₂₇ (tetradecanoic acid amide),
NH₂[(CH₂)ₓ₂NH]_{y1}COC₁₅H₃₁ (palmitic acid amide),
NH₂[(CH₂)ₓ₂NH]_{y1}COC₁₇H₃₅ (stearic acid amide),
NH₂[(CH₂)ₓ₂NH]_{y1}COC₁₇H₃₃ (oleic acid amide),
NH₂[(CH₂)ₓ₂NH]_{y1}COC₁₇H₃₃O (ricinolic acid amide),
NH₂[(CH₂)ₓ₂NH]_{y1}COC₁₇H₃₁ (linoleic acid amide),and
NH₂[(CH₂)ₓ₂NH]_{y1}COC₂₁H₄₁ (erucic acid amide),
wherein x2 is an integer of from 2 to 4, and y1 is an integer of from 2 to 8, and further preferably, x2 is 2,and y1 is an integer of from 2 to 5. Namely, the further preferred component (b) comprises one or more of the following amidates:

NH₂CH₂CH₂NHCH₂CH₂NHCOC₇H₁₅,

NH₂CH₂CH₂NHCH₂CH₂NHCOC₈H₁₇,

NH₂CH₂CH₂NHCH₂CH₂NHCOC₉H₁₉,

NH₂CH₂CH₂NHCH₂CH₂NHCOC₁₁H₂₃,

NH₂CH₂CH₂NHCH₂CH₂NHCOC₁₃H₂₇,

NH₂CH₂CH₂NHCH₂CH₂NHCOC₁₅H₃₁,

NH₂CH₂CH₂NHCH₂CH₂NHCOC₁₇H₃₅,

NH₂CH₂CH₂NHCH₂CH₂NHCOC₁₇H₃₃,

NH₂CH₂CH₂NHCH₂CH₂NHCOC₁₇H₃₃O,

NH₂CH₂CH₂NHCH₂CH₂NHCOC₁₇H₃₁,

NH₂CH₂CH₂NHCH₂CH₂NHCOC₂₁H₄₁,

NH₂CH₂CH₂NHCH₂CH₂NHCH₂CH₂NHCOC₇H₁₅,

NH₂CH₂CH₂NHCH₂CH₂NHCH₂CH₂NHCOC₈H₁₇,

NH₂CH₂CH₂NHCH₂CH₂NHCH₂CH₂NHCOC₉H₁₉,

NH₂CH₂CH₂NHCH₂CH₂NHCH₂CH₂NHCOC₁₁H₂₃,

NH₂CH₂CH₂NHCH₂CH₂NHCH₂CH₂NHCOC₁₃H₂₇,

NH₂CH₂CH₂NHCH₂CH₂NHCH₂CH₂NHCOC₁₅H₃₁,

NH₂CH₂CH₂NHCH₂CH₂NHCH₂CH₂NHCOC₁₇H₃₅,

NH₂CH₂CH₂NHCH₂CH₂NHCH₂CH₂NHCOC₁₇H₃₃,

NH₂CH₂CH₂NHCH₂CH₂NHCH₂CH₂NHCOC₁₇H₃₃O,

NH₂CH₂CH₂NHCH₂CH₂NHCH₂CH₂NHCOC₁₇H₃₁,

NH₂CH₂CH₂NHCH₂CH₂NHCH₂CH₂NHCOC₂₁H₄₁,

NH₂CH₂CH₂NHCH₂CH₂NHCH₂CH₂NHCH₂CH₂NHCOC₇H₁₅,

NH₂CH₂CH₂NHCH₂CH₂NHCH₂CH₂NHCH₂CH₂NHCOC₈H₁₇,

NH₂CH₂CH₂NHCH₂CH₂NHCH₂CH₂NHCH₂CH₂NHCOC₉H₁₉,

NH₂CH₂CH₂NHCH₂CH₂NHCH₂CH₂NHCH₂CH₂NHCOC₁₁H₂₃,

NH₂CH₂CH₂NHCH₂CH₂NHCH₂CH₂NHCH₂CH₂NHCOC₁₃H₂₇,

NH₂CH₂CH₂NHCH₂CH₂NHCH₂CH₂NHCH₂CH₂NHCOC₁₅H₃₁,

NH₂CH₂CH₂NHCH₂CH₂NHCH₂CH₂NHCH₂CH₂NHCOC₁₇H₃₅,

NH₂CH₂CH₂NHCH₂CH₂NHCH₂CH₂NHCH₂CH₂NHCOC₁₇H₃₃,

NH₂CH₂CH₂NHCH₂CH₂NHCH₂CH₂NHCH₂CH₂NHCOC₁₇H₃₃O,

NH₂CH₂CH₂NHCH₂CH₂NHCH₂CH₂NHCH₂CH₂NHCOC₁₇H₃₁,

NH₂CH₂CH₂NHCH₂CH₂NHCH₂CH₂NHCH₂CH₂NHCOC₂₁H₄₁,

NH₂CH₂CH₂NHCH₂CH₂NHCH₂CH₂NHCH₂CH₂NHCH₂CH₂NHCOC₁₁H₂₃,

NH₂CH₂CH₂NHCH₂CH₂NHCH₂CH₂NHCH₂CH₂NHCH₂CH₂NHCOC₁₃H₂₇,

NH₂CH₂CH₂NHCH₂CH₂NHCH₂CH₂NHCH₂CH₂NHCH₂CH₂NHCOC₁₅H₃₁,

NH₂CH₂CH₂NHCH₂CH₂NHCH₂CH₂NHCH₂CH₂NHCH₂CH₂NHCOC₁₇H₃₅,

NH₂CH₂CH₂NHCH₂CH₂NHCH₂CH₂NHCH₂CH₂NHCH₂CH₂NHCOC₁₇H₃₃,

NH₂CH₂CH₂NHCH₂CH₂NHCH₂CH₂NHCH₂CH₂NHCH₂CH₂NHCOC₁₇H₃₁,

and

(NH₂CH₂CH₂)₅NHCOC₁₇H₃₃O.

Said derivatives of polyamines can also be the reaction products of the condensation reaction of the above-mentioned polyamines with C1-C6 aldehyde. The condensation reaction of polyamines with aldehydes is commonly known in the art. The products are predominantly substituted triazines or substituted methanes. The reaction conditions generally include a molar ratio of total polyamines to C1-C6 aldehyde of 1: (0.1-10), preferably 1: 0.2-5, and more preferably 1: 0.3-3, in no presence of a solvent or at the present of a solvent, which is a hydrocarbon solvent, such as hexane, heptane, toluene, or xylene, added for refluxing and separating the reaction water, at a temperature of typically 80-150 °C, for a period of time such that the reaction no longer generates water, which is generally from 30 minutes to 10 hours. Said C1-C6 aldehyde is one or more of formaldehyde, acetaldehyde, propionaldehyde, butyraldehyde, valeraldehyde, caproaldehyde, cyclohexanecarboxaldehyde and an aqueous solution of one or more of them, and preferably one or more of formaldehyde, acetaldehyde, propionaldehyde, cyclohexanecarboxaldehyde and an aqueous solution of one or more of them. Said formaldehyde may be in the form of a formaldehyde solution or a polyformaldehyde.

Said derives of polyamines can also be the reaction products of the ammonolysis reaction of an acylating agent containing two acyl groups (C=O) in a molecule with the above-mentioned polyamines in a molar ratio of 1: (0.5-2), wherein said acylating agent containing two acyl groups in a molecule is one or more of a C6-C30 hydrocarbyl substituted organic dicarboxylic acid, a C6-C30 hydrocarbyl substituted anhydride, and a C6-C30 hydrocarbyl substituted half ester. Said ammonolysis reaction refers to a metathetic reaction of one or more of fatty acids, fatty acyl halides and fatty acid alkyl esters with polyamine to produce an amide. The reaction product of the above reaction can be used directly as component (b) without being isolated and purified, or the amidate alone therein can be used as component (b) after isolation and purification. Without isolation and purification, the mixture primarily comprises an amidate, and typically further comprises some unreacted starting materials and other reaction products, such as ammonium salts or alcohols. The specific composition of the mixture varies slightly depending on the reaction conditions.

In the present invention, the C6-C30 hydrocarbyl substituted organic dicarboxylic acid may be one or more of C6-C30 hydrocarbyl substituted maleic acid, butane dicarboxylic acid (succinic acid), fumaric acid, itaconic acid, citraconic acid, isatoic acid, and phthalic acid; the C6-C30 hydrocarbyl substituted anhydride may be one or more of C6-C30 hydrocarbyl substituted maleic anhydride, succinic anhydride (butane dicarboxylic acid anhydride), itaconic anhydride, citraconic anhydride, isatoic anhydride and phthalic anhydride; the C6-C30 hydrocarbyl substituted half ester may be a partially esterified product of the above C6-C30 hydrocarbyl substituted organic dicarboxylic acid or hydride with an alcohol, preferably a fatty alcohol. That is, a product is obtained by the esterification reaction of one of the two carbonyl groups in the organic dicarboxylic acid or anhydride with the alcohol, while the other carbonyl group does not take part in the esterification reaction. In the present invention, the preferred acylating agent containing two acyl groups in a molecule is one or more of C6-C30 hydrocarbyl substituted succinic acid and C6-C30 hydrocarbyl substituted succinic anhydride. Preferably, the structural formula of the C6-C30 hydrocarbyl substituted succinic acid is shown by formula (B3), and the structural formula of the C6-C30 hydrocarbyl substituted succinic anhydride is shown by formula (B4): wherein R is a hydrocarbyl having 6 to 30 carbon atoms. The term "hydrocarbyl" used herein is as defined above, and refers to hydrocarbon substituents, including aliphatic, alicyclic, aryl and heterocyclic substituents. The aliphatic hydrocarbyl may be a saturated hydrocarbyl or unsaturated hydrocarbyl having a double or triple bond. R is preferably an aliphatic hydrocarbyl having 8 to 24 carbon atoms, especially linear alkyl or alkenyl.

Representative C6-C30 hydrocarbyl substituted organic dicarboxylic acids useful as acylating agents in the present invention may be one or more of nonylsuccinic acid, decylsuccinic acid, dodecylsuccinic acid, tridecylsuccinic acid, tetradecylsuccinic acid, pentadecylsuccinic acid, hexadecylsuccinic acid, octadecylsuccinic acid, nonenylsuccinic acid, decenylsuccinic acid, dodecenylsuccinic acid, tetradecenylsuccinic acid, cetenylsuccinic acid, octadecenesuccinic acid, and docosenylsuccinic acid.

Representative C6-C30 hydrocarbyl substituted anhydrides useful as acylating agents in the present invention may be one or more of nonylsuccinic anhydride, decylsuccinic anhydride, dodecylsuccinic anhydride, tridecylsuccinic anhydride, tetradecylsuccinic anhydride, pentadecylsuccinic anhydride, hexadecylsuccinic anhydride, octadecylsuccinic anhydride, nonenylsuccinic anhydride, decenylsuccinic anhydride, dodecenylsuccinic anhydride, tetradecenylsuccinic anhydride, cetenylsuccinic anhydride, octadecenesuccinic anhydride, and docosenylsuccinic anhydride.

The process for preparing the above-mentioned C6-C30 hydrocarbyl substituted succinic anhydride is commonly known in the art, such as the thermal polymerization of a polyolefin having a corresponding chain length with maleic anhydride, or the substitution of a chlorinated hydrocarbon, e.g., a chlorinated polyolefin, with maleic anhydride. Please refer to US3361673, US3676089 and US3172892 for details.

The above-mentioned hydrocarbyl substituted succinic acid is commercially available or obtainable by a variety of methods known in the art, such as by hydrolysis of the corresponding hydrocarbyl substituted succinic anhydride by treating it with water or water vapor. Specific conditions and operations for hydrolysis are known by the person skilled in the art.

The ammonolysis reaction of the above-mentioned hydrocarbyl substituted succinic acid and/or succinic anhydride with a polyamine is commonly known in the art, and will not be described herein for details.

The reaction product of the ammonolysis reaction of a hydrocarbyl substituted succinic acid and/or succinic anhydride with a polyamine is related to both the reaction temperature and the molar ratio of the reactants. Generally speaking, a low reaction temperature (about 100 °C) results in the production of a product with predominant amide; a high reaction temperature (about 150 °C) results in the production of a product with predominant imide. In excess succinic acid and/or succinic anhydride, two or more succinic acid and/or succinic anhydride molecules react with the same polyamine molecule to produce the so-called "double hanging" or "multiple hanging" reaction product. The present invention preferably involves excess polyamine, which results in the production of a "mono-hanging" reaction product.

### Component (c)

Preferably, the additive composition of the present invention further comprises component (c), which is a metal deactivator capable of reacting with a metal surface and/or a metal chelator capable of reacting with or binding to a metal or metal ion. The weight ratio of said component (a) to said component (c) is 1: 0-1, preferably 1: 0.01-1, further preferably 1: 1: 0.01-0.5, and even further preferably 1: 0.02-0.2.

Specifically, said component (c) may be one or more of benzotriazole and derivatives thereof, thiadiazole and derivatives thereof, 8-hydroxyquinoline, ethylene diamine tetracarboxylic acids, hydrazides, β-diones, β-ketone esters, Schiff's bases, and organic polycarboxylic acid and derivatives thereof. Since benzotriazole does not have an excellent solubility in biodiesel, it is generally modified by, basically, introduction thereto of an oil soluble group, such as a long-chain hydrocarbyl, in order to increase its solubility in biodiesel. Thus, said benzotriazole derivatives may be various derivatives having a better solubility in biodiesel than benzotriazole. Specifically, said benzotriazole derivative may be one or more of an ammonium salt formed by benzotriazole and a fatty amine, and a product obtained by the Mannich reaction of benzotriazole, formaldehyde and a fatty amine. Said ethylene diamine tetracarboxylic acids may be ethylene diamine tetraacetic acid (EDTA), said hydrazides may be N-salicylidene-N'-salicyl hydrazide and/or N,N'-diacetyladipoyl dihydrazide. Said β-dione is, for example, acetylacetone, and said β-ketone ester is, for example, octylacetoacetate. Said Schiff's base may be one or more of N,N'-disalicylidene-1,2-ethylene diamine, N,N'-disalicylidene -1,2-propylene diamine, N,N'-disalicylidene-1,2-cyclohexanediamine, and N,N'-disalicylidene-N'-methyldipropylene triamine. Said organic polycarboxylic acid and derivatives thereof may be, for example, one or more of citric acid, tartaric acid, malic acid, succinic acid (butane dicarboxylic acid), maleic acid, phytic acid and derives thereof.

In the present invention, said component (c) is preferably one or more of benzotriazole, an ammonium salt formed from benzotriazole and a fatty amine, a product obtained by the Mannich reaction of benzotriazole, formaldehyde and a fatty amine (such as the commercially available additive T551), Schiff's base, organic polycarboxylic acids, and a product obtained by the condensation reaction of an organic polycarboxylic acid with a fatty amine or fatty alcohol (i.e., the amide or ester derivatives of organic polycarboxylic acids).

The additive composition of the present invention may further comprise one or more additional additives, such as flow improvers, cetane number improvers, antistatic agents, preservatives, rust inhibitors, and demulsifiers, if needed.

The preparation of the additive composition of the present invention is simple, only requiring the mixing of the components for forming the additive composition homogeneously. These components may be mixed directed or in the presence of a solvent, which can be a polar solvent, such as one or more of N,N-dimethylformamide (DMF), 1,4-dioxane, tetrahydrofuran (DHF), dimethyl sulphoxide (DMSO), pyrrolidone and methylpyrrolidone, or a hydrocarbon, in particularly an aromatic, such as benzene, toluene, xylene, an aromatic diluent oil and a mixture thereof and which can also be a biodiesel or a fatty alcohol, such as iso-octanol.

The diesel composition of the present invention can be obtained by adding an additive composition according to the present invention into a base diesel, or by adding each of the components of additives according to the present invention into a base diesel, respectively.

In the diesel composition of the present invention, the base diesel may be a pure biodiesel. Said biodiesel refers to the fatty acid low-carbon alcohol esters produced by the transesterification (alcoholysis) of oils/fats with low-carbon alcohols (such as C₁-C₅ fatty alcohols), and is commonly fatty acid methyl ester, i.e., a product of transesterification of an oil/fat with methanol.

Said transesterification may be any known or unknown process for the preparation of a biodiesel by the transesterification of an oil/fat with a low-carbon alcohol, such as, acid catalysis, base catalysis, enzyme catalysis, supercritical method and the like. Please refer to CN1473907A, DE3444893, CN1472280A, CN1142993C, CN1111591C and CN1594504A for details.

Said oil/fat has a generally recognized meaning in the art, is a general term for oils and fats, and comprises fatty acid triglyceride as the main component. Generally, those that are liquid at ambient temperature are called oils, and those that are solid or semi-solid at ambient temperature are called fats. Said oils/fats include vegetable oils and animal fats, and additionally, oil materials from microorganisms and algae, and can even be waste oils/fats, such as used or deteriorated oils/fats including used cooking oils, sewer oils, garbage oils, and acidified oils from oil/fat factories. Said vegetable oils may be oils from both herbs and woody plants, such as peanut oil, corn oil, cottonseed oil, rape seed oil, soybean oil, palm oil, safflower oil, flaxseed oil, coconut oil, oak oil, almond oil, walnut oil, castor oil, sesame oil, olive oil, Tall oil, sunflower oil, curcas oil, tung oil, sorbifolia oil, pistacia oil, and oils from halophytes, e.g., seaside mellow and cyperus beans. Said animal fats may be lard, chicken fat, duck fat, goose fat, mutton fat, horse fat, tallow, whale fat, shark fat, and the like.

In the biodiesel composition of the present invention, the base diesel may further comprise one or more additional diesels selected from the group consisting of petroleum diesel, Fischer-Tropsch synthetic diesel, hydrocracked biodiesel, and an oxygen-containing diesel concoction, wherein the ratio of the volume of said biodiesel to the volume of said additional diesels is preferably 1: 2-99.

Said petroleum diesel refers to a fuel for compression-ignited internal-combustion engines, obtained by subjecting a crude oil (petroleum) to various refining processes in a refinery, such as normal pressure-deduced process, catalytic cracking, catalytic reforming, carbonizing, hydrorefining, and hydrocracking, to produce a fraction having a distillation range between 160°C and 380 °C, and then formulating the fuel such that it will meet the national standard GB 252 for light diesels or the national standard GB 19147 for automobile diesels.

Fischer-Tropsch synthetic diesel primarily refers to GTL diesel (Gas To Liquid) or CTL diesel (Coal To Liquid) produced from natural gas or coal as the starting material, by Fischer-Tropsch (F-T) synthetic method, or BTL diesel (Biomass To Liquid) produce from plant fibers by Fischer-Tropsch synthetic method. Fischer-Tropsch synthetic diesel is substantially free of sulphur and aromatic hydrocarbon, and is a very clear fuel. However, it has a very poor lubricity. Though it has a greatly improved lubricity after being mixed with biodiesel, the oxidation stability of the blended oil may be deteriorated. Thus, a biodiesel-containing blended fuel requires the addition of antioxidants, too.

Hydrocracked biodiesel, also called second generation biodiesel, refers to the reaction products produced by the hydrogenation and cracking of animal fats and vegetable oils, which reaction products primarily comprise C₈-C₂₄ alkanes, in particular C₁₂-C₂₀ n-alkanes. Such hydrocracked biodiesel has a high hexadecane value but a low sulphur content and aromatic hydrocarbon content, and, when used as a fuel for diesel engines or as a blending component thereof, can greatly decrease the discharge of contaminants from diesel engines.

An oxygen-containing diesel blending component refers to an oxygen-containing compound or a mixture thereof that can be blended with various fuels for diesel engines to meet some standards or requirements. They are generally alcohols and ethers, or mixtures thereof. The alcohols may be, for example, C₁-C₁₈ fatty alcohols, preferably C₁-C₁₂ monofatty alcohols, such as methanol, ethanol, propanol, butanol, pentanol, hexanol, heptanol, octanol, nonanol, decanol, undecanol, lauryl alcohol and various isomers thereof. The ethers may be dimethylether, methyl tert-butylether, ethyl tert-butylether, C₆-C₁₄ fatty alcohol polyoxyvinylether, C₆-C₁₄ fatty alcohol polyoxypropene ether, C₆-C₁₄ alkylphenol polyoxyvinylether, C₆-C₁₄ alkylphenol polyoxypropene ether, polyoxymethylene dimethylether (CH₃O(CH₂O)ₓCH₃, wherein x=1-8) and mixtures thereof.

In the present invention, when the base diesel is a biodiesel-containing blended fuel, said diesel composition can be obtained by directly mixing the additives, biodiesel and additional diesels, or by first mixing the additives and biodiesel, and then blending them with the additional diesels. The additive components can be directly mixed with the ingredients of the base diesel, or can be premixed to obtain a mixture of additives which is subsequently mixed with the base diesel or the ingredients thereof. The additive components, the biodiesel and the additional diesels are mixed in an order which is not particularly defined, and namely, they can be mixed in various orders. The mixing can be performed at various conditions producing no detrimental effects on the additive composition and diesel composition, such as at ambient temperature.

The method of increasing the oxidation stability of biodiesel, according to the present invention, comprises blending an additive into a biodiesel-containing diesel component, wherein said additive is the above-mentioned additive composition of the present invention.

The present invention will be further exemplified by the following Examples.

Preparation Examples 1-6 are used for showing the preparation of the reaction product of the ammonolysis reaction of a polyamine with a monoacylating agent.

### Preparation Example 1

In a 500ml three-necked flask were added 100g lauric acid (0.5mol) and 56.7g tetraethylene pentamine (0.3mol), which were heated and stirred to 130 °C. Nitrogen gas was introduced and bubbled for 5 hours. 8.5g Water-like material was separated. By infrared analysis of the product, it was found out that the product had the characteristic peaks of amido groups (-CO-NH₂). Said reaction product was directly used as component (b).

### Preparation Example 2

Preparation Example 2 is the same as Preparation Example 1, except that the reactant contained 141.7g (0.75mol) tetraethylene pentamine. The reaction product was directly used as component (b).

### Preparation Example 3

In a 500ml three-necked flask were added 141g oleic acid (0.5mol), 77.4g N-(2-aminoethyl) piperazine (0.3mol) and 150g toluene, which were heated and stirred with refluxing and water separation for 6 hours. 8.3g Water-like material was separated, which was subjected to reduced pressure distillation to remove toluene and obtain a reaction product. By infrared analysis of the product, it was found out that the product had the characteristic peaks of amido groups. Said reaction product was directly used as component (b).

### Preparation Example 4

In a 250ml three-necked flask were added 100g dimer acid (an acid number of 197mg KOH/g, a YH13-type high-purity dimer acid produced by YUANDA CHEMICALS CO., LTD., Yichun, Jiangxi Province) and 82.0g pentaethylene hexamine (in a molar ratio of the carboxyl of the dimer acid to pentaethylene hexamine of 1: 1, with the carboxyl of the dimer acid calculated on the basis of the acid number), which were heated and stirred to 140 °C. Nitrogen gas was introduced and bubbled to separate reaction water for 4 hours to obtain a reaction product. By infrared analysis of the product, it was found out that the product had the characteristic peaks of amido groups. Said reaction product was directly used as component (b).

### Preparation Example 5

In a 250ml three-necked flask were added 100g tall oil fatty acid (an acid number of 190mg KOH/g, produced by Arizona) and 59.4g tri-(2-aminoethyl) amine (in a molar ratio of the carboxyl of the tall oil fatty acid to tri-(2-aminoethyl) amine of 1: 1.2, with the carboxyl of the tall oil fatty acid calculated on the basis of the acid number), which were heated and stirred to 120 °C. Nitrogen gas was introduced and bubbled to remove reaction water for 6 hours to obtain a reaction product. By infrared analysis of the product, it was found out that the product had the characteristic peaks of amido groups. Said reaction product was directly used as component (b).

### Preparation Example 6

In a 250ml three-necked flask were added 100g cottonseed oil biodiesel (produced by Shijiazhuang Refining and Chemical Branch of Sinopec), 24.7g triethylene tetramine and 21.8g N-(2-aminoethyl) piperazine (in a molar ratio of the fatty acid methylester of the biodiesel to triethylene tetramine to N-(2-aminoethyl) piperazine of about 1: 0.5: 0.5), which were heated to 120 °C. Nitrogen gas was introduced and bubbled with methanol for 8 hours to obtain a reaction product. Said reaction product was directly used as component (b).

Preparation Examples 7-10 are used for showing the synthesis of the condensation product of a polyamine with an aldehyde.

### Preparation Example 7

In a 500ml three-necked flask were added 56.7g tetraethylene pentamine (0.3mol), 38.7g N-(2-aminoethyl) piperazine (0.3mol) and 100g toluene, which were heated and stirred with refluxing. 42.0g formaldehyde solution having a concentration of 36 wt.% (0.5mol) was dropwisely added into the three-necked flask over a period of 2 hours. Refluxing and water separation were performed until no water was discharged (about 2 hours). After toluene was removed by reduced pressure distillation, 101g residue was obtained, which was blended with 105g aromatic diluent oil having a distillation range of 159-185 °C to form a diluent. Said diluent was directly used as component (b).

### Preparation Example 8

In a 500ml three-necked flask were added 69.6g pentaethylene hexamine (0.3mol), 9.0g polyformaldehyde (0.3mol, formaldehyde) and 80g toluene, which were heated and stirred with refluxing and water separation until no water was discharged (about 5 hours). After toluene was removed by reduced pressure distillation, 73g residue was obtained, which was blended with 73g aromatic diluent oil having a distillation range of 159-185 °C to form a diluent. Said diluent was directly used as component (b).

### Preparation Example 9

In a 500ml three-necked flask were added 43.8g triethylene tetramine (0.3mol), 72.6g N-dodecyl-1,3-propylene diamine (0.3mol), 18.0g polyformaldehyde (0.6mol, formaldehyde) and 125g toluene, which were heated and stirred with refluxing and water separation until no water was discharged (about 5 hours). After toluene was removed by reduced pressure distillation, 124g residue was obtained, which was blended with 120g aromatic diluent oil having a distillation range of 159-185 °C to form a diluent. Said diluent was directly used as component (b).

### Preparation Example 10

In a 500ml three-necked flask were added 56.7g tetraethylene pentamine (0.3mol), 43.5g N,N-bis-(3-aminopropyl) methylamine (0.3mol) and 110g toluene, which were heated and stirred with refluxing. 29.2g formaldehyde solution having a concentration of 36 wt.% (0.35mol) was dropwisely added into the three-necked flask over a period of 1 hour. Refluxing and water separation were then performed until no water was discharged (about 3 hours). The reaction product was directly used as component (b).

Preparation Examples 11-15 are used for showing the synthesis of the acylated product of a polyamine.

### Preparation Example 11

In a 500ml three-necked flask were added 56.7g tetraethylene pentamine (0.3mol), 96.5g hexadecenylsuccinic anhydride (0.3mol) and 136.5g xylene, which were heated and stirred with refluxing and water separation for 5 hours. About 5g water was separated, resulting in a mixture comprising about 50 wt.% of an ammonolysis reaction product comprising predominantly hexadecenylsuccinimide. The mixture was directly used as component (b).

### Preparation Example 12

In a 500ml three-necked flask were added 46.4g pentaethylene hexamine (0.2mol), 25.8g N-(2-aminoethyl) piperazine (0.2mol), 56.8g dodecenylsuccinic acid (0.2mol) and 130g toluene, which were heated and stirred with refluxing and water separation for 6 hours. Toluene was removed by reduced pressure distillation, resulting in 121g ammonolysis reaction product comprising predominantly dodecenylsuccinic amide. Said ammonolysis reaction product was further blended with 123g aromatic diluent oil having a distillation range of 159-185 °C to form a diluent. Said diluent was directly used as component (b).

### Preparation Example 13

In a 500ml three-necked flask were added 100g dodecenylsuccinic acid half ester (an additive product with the trade name T747, produced by Lushun Chemical Plant, with an acid number of about 180mg KOH/g), 46.9g triethylene tetramine (in a molar ratio of triethylene tetramine to the carboxyl of the dodecenylsuccinic acid half ester of 1: 1, calculated on the basis of the acid number of T747), and 150g aromatic diluent oil having a distillation range of 159-185 °C, which were heated and stirred. Nitrogen gas was used for bubbling to remove reaction water at 110 °C for 5 hours. About 5g water was separated. The resultant product was directly used as component (b).

### Preparation Example 14

In a 500ml three-necked flask were added 56.7g tetraethylene pentamine (0.3mol), 79.8g dodecenylsuccinic anhydride (0.3mol), and 136.5g aromatic diluent oil having a distillation range of 159-185 °C, which were heated and stirred. Nitrogen gas was used for bubbling to remove reaction water at 150 °C for 5 hours. About 5g water was separated, resulting in a mixture comprising about 50 wt.% of an ammonolysis reaction product comprising predominantly mono-dodecenylsuccinimide. The mixture was directly used as component (b).

### Preparation Example 15

The process of Preparation Example 14 was conducted, except that 28.4g tetraethylene pentamine (0.15mol) was used for replacing 56.7g tetraethylene pentamine (0.3mol), and 108.2g aromatic diluent oil having a distillation range of 159-185 °C was used for replacing 136.5g aromatic diluent oil having a distillation range of 159-185 °C. A mixture comprising about 50 wt.% of an ammonolysis reaction product comprising predominantly bis-dodecenylsuccinimide was obtained. Said mixture was directly used as component (b).

The following Examples are used for showing the preparation of the additives in the diesel composition of the present invention.

### Examples 1-9

Examples 1-9 demonstrate the preparation of the additive composition of the present invention, wherein component (b) was a polyamine.

Components (a), (b) and (c) were mixed according to the weight ratios shown in Table 1.

**Table 1**

| Example | component (a) | component (b) | component (c) | a:b:c (weight ratio) |
|---|---|---|---|---|
| Example 1 | N,N'-di-sec-butyl-p-phenylene diamine | Tri- (2 - amino ethyl) amine | - | 1:4:0 |
| Example 2 | Antioxidant 88 | N-cocoyl-1,3-propylene diamine | - | 1:1.2:0 |
| Example 3 | N,N'-di-sec-butyl-p-phenylene diamine | Tetraethylene pentamine | - | 1:1:0 |
| Example 4 | N,N'-di-sec-butyl-p-phenylene diamine | Tetraethylene pentamine | N,N'-disalicylidene -1,2-propylene diamine | 1:1:0.06 |
| Example 5 | Antioxidant 4020 | N,N-dimethyl-1,3-propylene diamine | - | 2:1:0 |
| Example 6 | N,N'-bis-(1-methylheptyl) p-phenylene diamine (antioxidant 288) | Polyether diamine (CAS No. 9046-10-0) | - | 1:2:0 |
| Example 7 | Antioxidant 88 | N-(2-aminoethyl) piperazine | - | 1:0.2:0 |
| Example 8 | Antioxidant 688 | N,N-bis-(3-aminopropyl) methylamine | - | 1:0.5:0 |
| Example 9 | N,N'-di-sec-butyl-p-phenylene diamine | N-(2-aminoethyl) piperazine | - | 1:8:0 |

Either component (a) or component (b) alone was used as a biodiesel antioxidant, was combined, according to the process of the present invention, with an organic amine beyond the scope of the amine of the present invention as component (b), forming the following comparative examples of the present invention:
Comparative Example a1: N,N'-di-sec-butyl-p-phenylene diamine;
Comparative Example b1: tri(2-aminoethyl) amine;
Comparative Example a2: antioxidant 88;
Comparative Example b2: N-cocoyl-1,3-propylene diamine;
Comparative Example b3: tetraethylene pentamine;
Comparative Example a3: antioxidant 4020;
Comparative Example b4: N,N-dimethyl-1,3-propylene diamine;
Comparative Example a4: N,N'-bis-(1-methylheptyl)p-phenylene diamine;
Comparative Example b5: polyether diamine (CAS No. 9046-10-0);
Comparative Example a5: antioxidant 688;
Comparative Example b6: N-(2-aminoethyl) piperazine;
Comparative Example b7: N,N-bis- (3-aminopropyl) methylamine;
Comparative Example 1: a combination of N,N'-di-sec-butyl-p-phenylene diamine with N,N-dimethylcyclohexylamine in a weight ratio of 1: 1;
Comparative Example 2: a combination of N,N'-di-sec-butyl-p-phenylene diamine with N,N,N',N'-tetramethyl-1,4-butane diamine in a weight ratio of 1: 1;
Comparative Example 3: a combination of N,N'-di-sec-butyl-p-phenylene diamine with triethylene diamine (TEDA) in a weight ratio of 1: 1.

### Examples 10-17

The following Examples demonstrate the preparation of the additive composition of the present invention, wherein component (b) was a polyamine derivative produced by the amination reaction of a monofatty acid or ester with a polyamine.

Components (a), (b) and (c) were mixed according to the weight ratios shown in Table 2.

**Table 2**

| Example | component (a) | component (b) | component (c) | a:b:c |
|---|---|---|---|---|
| Example 10 | N,N'-di-sec-butyl-p-phenylene diamine | Preparation Example 1 | - | 2:1:0 |
| Example 11 | N,N'-di-sec-butyl-p-phenylene diamine | Preparation Example 2 | - | 2:1:0 |
| Example 12 | Antioxidant 88 | Preparation Example 3 | - | 1:3:0 |
| Example 13 | Antioxidant 288 | Preparation Example 3 | - | 1:2:0 |
| Example 14 | N,N'-di-sec-butyl-p-phenylene diamine | Preparation Example 4 | - | 1:1:0 |
| Example 15 | N,N'-di-sec-butyl-p-phenylene diamine | Preparation Example 4 | N,N'-disalicylidene -1,2-propylene diamine | 1:1:0.0 6 |
| Example 16 | Antioxidant 688 | Preparation Example 5 | - | 3:1:0 |
| Example 17 | N,N'-di-sec-butyl-p-phenylene diamine | Preparation Example 6 | - | 1:5:0 |

Comparative Example b8: Preparation Example 1;
Comparative Example b9: Preparation Example 2;
Comparative Example b10: Preparation Example3;
Comparative Example b11: Preparation Example 4;
Comparative Example b12: Preparation Example 5;
Comparative Example b13: Preparation Example 6.

### Examples 18-24

Examples 18-24 demonstrate the preparation of the additive composition of the present invention, wherein component (b) was a polyamine derivative produced by the amination reaction of an aldehyde with a polyamine.

Components (a), (b) and (c) were mixed according to the weight ratios shown in Table 3.

**Table 3**

| Example | component (a) | component (b) | component (c) | a:b:c |
|---|---|---|---|---|
| Example 18 | N,N'-di-sec-butyl-p-phenylene diamine | Preparation Example 7 | - | 2:1:0 |
| Example 19 | Antioxidant 88 | Preparation Example 8 | - | 1:3:0 |
| Example 20 | N,N'-di-sec-butyl-p-phenylene diamine | Preparation Example 9 | - | 1:1:0 |
| Example 21 | N,N'-di-sec-butyl-p-phenylene diamine | Preparation Example 9 | Tartaric acid | 1:1:0.2 |
| Example 22 | Antioxidant 288 | Preparation Example 10 | - | 3:1:0 |
| Example 23 | 4,4'-dioctyldiphenyl amine | Preparation Example 7 | - | 2:1:0 |
| Example 24 | Antioxidant 688 | Preparation Example 9 | - | 1:1:0 |

Comparative Example b14: Preparation Example 7;
Comparative Example b15: Preparation Example 8;
Comparative Example b16: Preparation Example 9;
Comparative Example b17: Preparation Example 10;
Comparative Example a6: 4,4'-dioctyldiphenylamine.

### Examples 25-31

Examples 25-31 demonstrate the preparation of the additive composition of the present invention, wherein component (b) was a polyamine derivative produced by the amination reaction of a diacylating agent with a polyamine.

Components (a), (b) and (c) were mixed according to the weight ratios shown in Table 4.

**Table 4**

| Example | component (a) | component (b) | component (c) | a:b:c |
|---|---|---|---|---|
| Example 25 | Antioxidant 88 | Preparation Example 11 | - | 2:1:0 |
| Example 26 | 4,4'-dioctyldiphenyl amine | Preparation Example 11 | - | 2:1:0 |
| Example 27 | Antioxidant 288 | Preparation Example 13 | - | 1:4:0 |
| Example 28 | N,N'-di-sec-butyl-p-phenylene diamine | Preparation Example 12 | - | 1:1:0 |
| Example 29 | N,N'-di-sec-butyl-p-phenylene diamine | Preparation Example 12 | N,N'-disalicylidene -1,2-propylene diamine | 1:1:0.06 |
| Example 30 | Antioxidant 688 | Preparation Example 14 | - | 1:1:0 |
| Example 31 | Antioxidant 688 | Preparation Example 15 | | 1:1:0 |

Comparative Example b18: Preparation Example 11;
Comparative Example b19: Preparation Example 12;
Comparative Example b20: Preparation Example 13;
Comparative Example b21: Preparation Example 14;
Comparative Example b22: Preparation Example 15.

### Property Tests

In the following tests, the cottonseed oil biodiesel and rapeseed oil biodiesel were the products provided by Shijiazhuang Refining and Chemical Branch of Sinopec, the sewer oil biodiesel and acidified oil biodiesel were both provided by Longyan Zhuoyue New Energy Development Co., Ltd, Fujian, and the petroleum diesel was the diesel of Beijing Standard B produced by Sinopec Yanshan Branch.

### (1) Test on the oxidation stability of a biodiesel composition comprising pure biodiesel as base diesel

The oxidation stability of the biodiesel was tested by measuring its induction period at 110 °C using the EN14112:2003 method (Rancimat method) with an instrument of model 743 for measuring the oxidation stability of a fat or oil from Metrohm Schweiz AG. The longer the induction period is, the better the antioxidative property of the diesel composition; vice versa, the shorter the induction period is, the poorer the antioxidative property of the diesel composition. The results of the test were shown in Tables 5 to 8.

**Table 5**

| Biodiesel | Source of Additive | Amount Added/(mg/kg) | Induction Period at 110 °C/(hr) |
|---|---|---|---|
| Cottonseed Oil Biodiesel | - | - | 1.0 |
| | Example 1 | 500 | 21.4 |
| | Comparative Example a1 | 100 | 3.1 |
| | Comparative Example a1 | 500 | 9.8 |
| | Comparative Example b1 | 400 | 1.1 |
| | Comparative Example b1 | 500 | 1.6 |
| | Example 2 | 550 | 17.6 |
| | Comparative Example a2 | 250 | 5.9 |
| | Comparative Example a2 | 550 | 9.3 |
| | Comparative Example b2 | 300 | 0.9 |
| | Comparative Example b2 | 550 | 1.9 |
| | Example 3 | 400 | 18.4 |
| | Comparative Example a1 | 200 | 5.4 |
| | Comparative Example a1 | 400 | 9.0 |
| | Comparative Example b3 | 200 | 1.0 |
| | Comparative Example b3 | 400 | 3.1 |
| | Comparative Example 1 | 400 | 0.9 |
| | Example 4 | 412 | 20.5 |
| | Example 5 | 600 | 20.9 |
| | Comparative Example a3 | 400 | 8.5 |
| | Comparative Example a3 | 600 | 10.1 |
| | Comparative Example b4 | 200 | 0.9 |
| | Comparative Example b4 | 600 | 3.0 |
| | Example 6 | 750 | 22.1 |
| | Comparative Example a4 | 250 | 5.4 |
| | Comparative Example a4 | 750 | 11.1 |
| | Comparative Example b5 | 500 | 1.5 |
| | Comparative Example b5 | 750 | 3.1 |
| Sewer Oil Biodiesel | - | - | 0.9 |
| | Example 3 | 600 | 25.1 |
| | Comparative Example a1 | 300 | 6.7 |
| | Comparative Example al | 600 | 10.9 |
| | Comparative Example b3 | 300 | 1.0 |
| | Comparative Example b3 | 600 | 4.2 |
| | Comparative Example 2 | 600 | 1.2 |
| | Comparative Example 3 | 600 | 0.4 |
| | Example 7 | 600 | 20.4 |
| | Comparative Example a2 | 600 | 10.2 |
| | Comparative Example b6 | 100 | 1.0 |
| | Comparative Example b6 | 600 | 0.9 |
| | Example 8 | 750 | 29.8 |
| | Comparative Example a5 | 500 | 9.0 |
| | Comparative Example a5 | 750 | 12.8 |
| | Comparative Example b7 | 250 | 1.1 |
| | Comparative Example b7 | 750 | 4.9 |
| | Example 9 | 720 | 21.3 |
| | Comparative Example a1 | 720 | 12.2 |
| | Comparative Example b6 | 720 | 2.9 |

As can be seen from the data in Table 5, component (a) was a common antioxidant, which improved the oxidation stability of biodiesel in some degree, component (b) had no antioxidative effect or a relatively poor antioxidative effect when used alone, and component (a) and component (b) used alone were both listed as comparative examples of the present invention. The oxidation stability of the biodiesel compositions of the present invention were significantly improved. A biodiesel composition comprising a combination of component (a) with component (b) produced a much better effect than the sum of the effects produced by biodiesel compositions comprising component (a) or component (b) alone. Thus it can be seen that components (a) and (b) surprisingly produced an evident synergistic effect. The effect was further enhanced by the addition of an optional component (c).

Upon comparison of Example 3 with Example 4, it can be seen that the oxidation stability of a biodiesel composition comprising the optional component (c) was further enhanced.

Upon comparison of Comparative Examples 1, 2 and 3 with Example 3, it can be seen that the combination of an amine-type compound beyond the scope of the present invention as component (b) with an antioxidant of component (a) did not produce any synergism, and on the contrary, led to disappearance of the antioxidative effect, indicating the presence of antagonism. Component (b) in Comparative Example 1 was a mono-tertiary amine, and components (b) in Comparative Examples 2 and 3 were di-tertiary amines, in which the nitrogen atom was not linked to the hydrogen atom in the molecular structure.

**Table 6**

| Biodiesel | Source of Additive | Amount Added/(mg/kg) | Induction Period at 110 °C/(hr) |
|---|---|---|---|
| Cottonseed Oil Biodiesel | - | - | 1.0 |
| | Example 10 | 450 | 18.9 |
| | Comparative Example a1 | 450 | 9.2 |
| | Comparative Example b8 | 150 | 0.8 |
| | Comparative Example b8 | 450 | 2.8 |
| | Example 11 | 450 | 20.9 |
| | Comparative Example b9 | 150 | 0.8 |
| | Comparative Example b9 | 450 | 3.0 |
| | Example 12 | 600 | 16.8 |
| | Comparative Example a2 | 600 | 9.8 |
| | Comparative Example b10 | 450 | 0.8 |
| | Comparative Example b10 | 600 | 2.9 |
| | Example 13 | 600 | 21.4 |
| | Comparative Example a4 | 600 | 9.3 |
| | Comparative Example b10 | 400 | 0.8 |
| | Example 14 | 600 | 19.2 |
| | Example 15 | 618 | 22.8 |
| | Comparative Example a1 | 600 | 11.1 |
| | Comparative Example b11 | 400 | 0.8 |
| | Comparative Example b11 | 600 | 3.0 |
| Sewer Oil Biodiesel | - | - | 0.9 |
| | Example 10 | 600 | 25.4 |
| | Comparative Example a1 | 400 | 7.5 |
| | Comparative Example b8 | 200 | 1.0 |
| | Comparative Example b8 | 600 | 3.9 |
| | Example 16 | 400 | 18.2 |
| | Comparative Example a5 | 300 | 6.8 |
| | Comparative Example a5 | 400 | 8.3 |
| | Comparative Example b12 | 100 | 1.0 |
| | Comparative Example b12 | 400 | 3.3 |
| | Example 17 | 600 | 17.7 |
| | Comparative Example a1 | 100 | 3.4 |
| | Comparative Example a1 | 600 | 10.9 |
| | Comparative Example b13 | 500 | 0.9 |
| | Comparative Example b13 | 600 | 1.8 |

As can be seen from the data in Table 6, component (a) was a common antioxidant, which improved the oxidation stability of biodiesel in some degree, component (b) had no antioxidative effect or a relatively poor antioxidative effect when used alone, and component (a) and component (b) used alone were both listed as comparative examples of the present invention. The biodiesel composition of the present invention had a significantly improved oxidation stability, showing that a biodiesel composition comprising a combination of component (a) with component (b) produced a much better effect than the sum of the effects produced by biodiesel compositions comprising component (a) or component (b) alone. Thus it can be seen that components (a) and (b) surprisingly produced an evident synergistic effect. The effect was further enhanced by the addition of an optional component (c).

Upon comparison of Example 10 with Example 11, it can be seen that the reaction product resulting from excess amine during the preparation of component (b) produced a slightly better effect. Upon comparison of Example 14 with Example 15, it can be seen that the oxidation stability of a biodiesel composition comprising the optional component (c) was further enhanced.

**Table 7**

| Biodiesel | Source of Additive | Amount Added/(mg/kg) | Induction Period at 110 °C/(hr) |
|---|---|---|---|
| Cottonseed Oil Biodiesel | - | - | 1.0 |
| | Example 18 | 450 | 19.9 |
| | Comparative Example a1 | 300 | 7.2 |
| | Comparative Example a1 | 450 | 9.2 |
| | Comparative Example b14 | 150 | 1.0 |
| | Comparative Example b14 | 450 | 2.9 |
| | Example 19 | 400 | 16.2 |
| | Comparative Example a2 | 100 | 4.9 |
| | Comparative Example a2 | 400 | 8.0 |
| | Comparative Example b15 | 300 | 0.8 |
| | Comparative Example b15 | 400 | 1.7 |
| | Example 20 | 600 | 20.2 |
| | Example 21 | 660 | 25.0 |
| | Comparative Example a1 | 600 | 11.1 |
| | Comparative Example b16 | 300 | 1.0 |
| | Comparative Example b16 | 600 | 3.2 |
| | Example 22 | 600 | 22.9 |
| | Comparative Example a4 | 600 | 9.3 |
| | Comparative Example b17 | 150 | 0.9 |
| | Comparative Example b17 | 600 | 3.3 |
| | Example 23 | 450 | 6.3 |
| | Comparative Example a6 | 300 | 3.1 |
| | Comparative Example a6 | 450 | 4.0 |
| | Example 24 | 600 | 18.6 |
| | Comparative Example a5 | 300 | 6.5 |
| | Comparative Example a5 | 600 | 10.7 |
| Acidified Oil Biodiesel | - | - | 0.9 |
| | Example 18 | 600 | 25.4 |
| | Comparative Example a1 | 400 | 7.5 |
| | Comparative Example a1 | 600 | 10.3 |
| | Comparative Example b14 | 200 | 1.0 |
| | Comparative Example b14 | 600 | 3.8 |
| | Example 19 | 400 | 20.3 |
| | Comparative Example a2 | 100 | 4.5 |
| | Comparative Example a2 | 400 | 8.6 |
| | Comparative Example b15 | 300 | 1.9 |
| | Comparative Example b15 | 400 | 3.0 |
| | Example 23 | 600 | 8.5 |
| | Comparative Example a6 | 400 | 4.7 |
| | Comparative Example a6 | 600 | 5.8 |
| | Comparative Example b14 | 200 | 1.2 |
| | Comparative Example b14 | 600 | 3.8 |

As can be seen from the data in Table 7, component (a) was a common antioxidant, which improved the oxidation stability of biodiesel in some degree, and component (b) did not improve the antioxidative effect of biodiesel or had a very poor antioxidative effect when used alone in a small amount. The biodiesel composition of the present invention had a significantly improved oxidation stability. A biodiesel composition comprising a combination of component (a) with component (b) produced a much better effect than the sum of the effects produced by biodiesel compositions comprising component (a) or component (b) alone. Thus it can be seen that components (a) and (b) surprisingly produced an evident synergistic effect.

Upon comparison of Example 21 with Example 20, it can be seen that the oxidation stability of a biodiesel composition comprising the optional component (c) was further enhanced.

**Table 8**

| Biodiesel | Source of Additive | Amount Added/(mg/kg) | Induction Period at 110 °C/(hr) |
|---|---|---|---|
| Rapeseed Oil | - | - | 1.2 |
| | Example 25 | 600 | 23.8 |
| | Comparative Example a2 | 400 | 8.1 |
| | Comparative Example a2 | 600 | 10.4 |
| | Comparative Example b18 | 200 | 1.4 |
| | Comparative Example b18 | 600 | 3.6 |
| | Example 26 | 600 | 9.3 |
| | Comparative Example a6 | 400 | 4.2 |
| | Comparative Example a6 | 600 | 6.0 |
| | Example 27 | 750 | 22.1 |
| | Comparative Example a4 | 150 | 3.9 |
| | Comparative Example a4 | 750 | 9.1 |
| | Comparative Example b20 | 600 | 1.4 |
| | Comparative Example b20 | 750 | 2.6 |
| | Example 28 | 700 | 27.9 |
| | Example 29 | 721 | 31.2 |
| | Comparative Example a1 | 350 | 7.9 |
| | Comparative Example a1 | 700 | 14.4 |
| | Comparative Example b19 | 350 | 1.5 |
| | Comparative Example b19 | 700 | 5.2 |
| | Example 30 | 700 | 28.6 |
| | Comparative Example a5 | 350 | 7.0 |
| | Comparative Example a5 | 700 | 13.3 |
| | Comparative Example b21 | 350 | 1.3 |
| | Comparative Example b21 | 700 | 5.6 |
| | Example 31 | 700 | 17.7 |
| | Comparative Example b22 | 350 | 1.1 |
| | Comparative Example b22 | 700 | 4.2 |
| Sewer oil Biodiesel | - | - | 0.9 |
| | Example 27 | 750 | 29.2 |
| | Comparative Example a4 | 150 | 4.2 |
| | Comparative Example a4 | 750 | 12.1 |
| | Comparative Example b20 | 600 | 3.5 |
| | Comparative Example b20 | 750 | 4.9 |
| | Example 28 | 750 | 24.8 |
| | Comparative Example a1 | 400 | 7.5 |
| | Comparative Example a1 | 600 | 10.9 |
| | Comparative Example b19 | 600 | 3.7 |

As can be seen from the data in Table 8, component (a) was a common antioxidant, which improved the oxidation stability of biodiesel in some degree, and component (b) had no antioxidative effect or a relatively poor antioxidative effect when used alone. The biodiesel composition of the present invention had a significantly improved oxidation stability. A biodiesel composition comprising a combination of component (a) with component (b) produced a much better effect than the sum of the effects produced by biodiesel compositions comprising component (a) or component (b) alone. Thus it can be seen that components (a) and (b) surprisingly produced an evident synergistic effect. The effect was further enhanced by the addition of an optional component (c).

Upon comparison of Example 28 with Example 29, it can be seen that the oxidation stability of a biodiesel composition comprising the optional component (c) was further enhanced.

Upon comparison of Example 30 with Example 31, it can be seen that when component (b) was mono-alkenylsuccimide ("mono-hanging"), the combination of it with an antioxidant produced a better antioxidative effect than the combination of it with an antioxidant, when component (b) is bi-alkenylsuccimide ("double hanging").

The above oxidation stability data of additives were all obtained after three months from the production of the biodiesels. The effect of the present invention was more significant when a sewer oil biodiesel freshly produced (within one week) was used in the tests. Results were shown in Table 9.

**Table 9**

| Biodiesel | Source of Additive | Amount Added/(mg/kg) | Induction Period at 110 °C/(hr) |
|---|---|---|---|
| Freshly Produced Sewer Oil Biodiesel | - | - | 2.1 |
| | Example 3 | 500 | 39.8 |
| | Comparative Example a1 | 250 | 13.1 |
| | Comparative Example a1 | 500 | 19.7 |
| | Comparative Example b3 | 250 | 3.8 |
| | Comparative Example b3 | 500 | 6.3 |
| | Example 9 | 720 | 44.9 |
| | Comparative Example a1 | 80 | 5.1 |
| | Comparative Example a1 | 720 | 22.7 |
| | Comparative Example b6 | 640 | 5.9 |
| | Comparative Example b6 | 720 | 6.2 |

As can be seen from Table 9, the freshly produced biodiesel was more susceptible to the antioxidant formulation of the present invention. It can be seen from Example 9 and its Comparative Examples that the use of a polyamine-type compound in the present invention greatly reduced the amount of an arylamine-type antioxidant which has some toxicity and dyeability, but produced a greatly improved effect than the arylamine-type antioxidant.

### (2) Tests on the antioxidative property and oxidation stability of a blended diesel composition comprising biodiesel and petroleum diesel as base diesel, wherein the biodiesel was sewer oil biodiesel

The induction periods of the diesel compositions, petroleum diesel and blended diesels at 110 °C were independently measured by the Pr EN15751:2008 method were measured with using a tester of model 743 for measuring the oxidation stability of a fat or oil from Metrohm Schweiz AG. The longer the induction period is, the better the antioxidative property of the diesel composition; vice versa, the shorter the induction period is, the poorer the antioxidative property of the diesel composition. The results of the test were shown in Tables 10 to 13.

The amount of total insolubles (unit: mg/100 mL) in the blended diesel compositions was measured using the SH/T 0175 method, so as to assess the stability of the diesel compositions. The larger the amount of total insolubles is, the poorer the stability; vice versa, the smaller the amount of total insolubles is, the better the stability. The results of the test were shown in Tables 10 to 13.

**Table 10**

| Base Diesel | Source of Additive | Amount Added (mg/kg) | Oxidation Stability, Induction Period (110 °C)/hr | Stability, Total Insolubles (mg/100 mL) |
|---|---|---|---|---|
| Petroleum Diesel | - | - | >50 | 0.5 |
| Petroleum Diesel: Biodiesel = 80: 20 (volume) (B20) | - | - | 5.8 | >10 |
| | Example 3 | 200 | >50 | 3.1 |
| | Comparative Example a1 | 200 | 34.2 | 6.4 |
| | Comparative Example b3 | 200 | 7.9 | >10 |
| | Example 5 | 300 | >50 | 2.0 |
| | Comparative Example a3 | 200 | 36.1 | 4.8 |
| | Comparative Example b4 | 100 | 5.6 | >10 |

**Table 11**

| Base diesel | Source of Additive | Amount Added (mg/kg) | Oxidation Stability, Induction Period (110 °C)/hr | Stability, Total Insolubles (mg/100 mL) |
|---|---|---|---|---|
| Petroleum Diesel | - | - | >50 | 0.5 |
| Petroleum Diesel: Biodiesel = 85:15 (volume) (B15) | - | - | 7.2 | 8.8 |
| | Example 14 | 200 | >50 | 1.5 |
| | Comparative Example a1 | 200 | 32.1 | 5.1 |
| | Comparative Example b11 | 200 | 6.6 | 9.0 |

**Table 12**

| Base Diesel | Source of Additive | Amount Added (mg/kg) | Oxidation Stability, Induction Period (110 °C)/hr | Stability, Total Insolubles (mg/100 mL) |
|---|---|---|---|---|
| Petroleum Diesel | - | - | >50 | 0.5 |
| Petroleum Diesel: Biodiesel = 85: 15 (volume) (B15) | - | - | 4.2 | 8.8 |
| | Example 20 | 200 | >50 | 2.5 |
| | Comparative Example a1 | 200 | 32.1 | 5.1 |
| | Comparative Example b16 | 200 | 4.6 | 9.0 |
| | Example 20 | 90* | >50 | 4.8 |

| | | | | |
|---|---|---|---|---|
| * The amount of additive was calculated as 90 mg/kg in the blended fuel which was obtained by blending a biodiesel, in which the additive of Example 20 had been added in an amount of 600 mg/kg, with petroleum diesel in a ratio of 15: 85 by volume. | | | | |

**Table 13**

| Base Diesel | Source of Additive | Amount Added (mg/kg) | Oxidation Stability, Induction Period (110 °C)/hr | Stability, Total Insolubles (mg/100 mL) |
|---|---|---|---|---|
| Petroleum Diesel | - | - | >50 | 0.5 |
| Petroleum Diesel: Biodiesel = 85: 15 (volume) (B15) | - | - | 4.5 | 8.9 |
| | Example 28 | 200 | >50 | 1.3 |
| | Comparative Example a1 | 200 | 41.8 | 5.4 |
| | Comparative Example bl9 | 200 | 4.6 | 8.7 |
| | Example 28 | 90* | >50 | 3.4 |

| | | | | |
|---|---|---|---|---|
| * The amount of additive was calculated as 90 mg/kg in the blended fuel which was obtained by blending a biodiesel, in which the additive of Example 31 had been added in an amount of 600 mg/kg, with petroleum diesel in a ratio of 15: 85 by volume. | | | | |

As can be seen from the results of Tables 10 to 13, the blended fuels comprising biodiesel all had deteriorated oxidation stability and stability than petroleum diesel. However, the biodiesel composition comprising a mixture of component (a) and component (b) as additive had significantly improved oxidation stability and stability, and components (a) and (b) exhibited synergism, i.e., a significantly enhanced effect, compared with the use of one of them alone.

## Claims

1. A diesel composition, which comprises a base diesel and an additive composition, **characterized in that** said base diesel comprises biodiesel, and said additive composition comprises component (a) and component (b), wherein said component (a) is a substituted p-phenylene diamine, and said component (b) is one or more polyamines or derivatives thereof, wherein the polyamine is a polyether diamine of formula (A1):
wherein x1 is an integer from 1 to 10, R₄ is H or a hydrocarbyl having 1 to 30 carbon atoms, and R₅ is H or methyl: or a polyene polyamine of the structural formula:
H₂N[(CH₂)ₓ₂NH]_{y1}R₆
wherein x2 is an integer from 2 to 4, y1 is an integer from 1 to 8, and R₆ is H or a hydrocarbyl having 1 to 30 carbon atoms, and/or a condensate of said polyene polyamine with ethylene oxide and/or propylene oxide; or
an imidazoline-type polyamine of the formula (A2);
wherein y2 is an integer from 0 to 5, and R₇ is a hydrocarbyl having 1 to 24 carbon atoms; or
a piperazine-type polyamine being N-(2-aminoethyl)piperazine or N,N'-di-(aminoethyl)piperazine; or
a piperidine-type polyamine: or
a tertiary amine containing polyamine of the formula (A₄), (A₅) or (A6):
wherein R₉ and R₁₀ are hydrocarbyls having 1 to 24 carbon atoms, and x4 is an integer from 0 to 10; or
wherein x5 is an integer from 1 to 10; or
wherein R₁₁ is a hydrocarbyl having 1 to 24 carbon atoms, and x6 is an integer from 1 to 10, and preferably an integer from 2 to 6;
wherein said derivatives of polyamines are the reaction products of the ammonolysis reaction of one or more organic acids having 6 to 40 carbon atoms, acyl halides having 6 to 40 carbon atoms, or organic acid alkyl esters having 6 to 40 carbon atoms with the above-mentioned polyamines, or
wherein said derivatives of polyamines are the reaction products of the condensation reaction of said polyamines with C1-C6 aldehyde, or
wherein said derivatives of polyamines are the reaction products of the ammonolysis reaction of an acylating agent containing two acyl groups in a molecule with the above-mentioned polyamines in a molar ratio of 1: (0.5-2), wherein said acylating agent containing two acyl groups in a molecule is one or more of a C6-C30 hydrocarbyl substituted organic dicarboxylic acid, a C6-C30 hydrocarbyl substituted anhydride, and a C6-C30 hydrocarbyl substituted half ester; and wherein the weight ratio of said component (b) to said component (a) is 0.01-100:1 .

2. The diesel composition according to claim 1, wherein the weight ratio of said component (b) to said component (a) is 0.05-10:1.

3. The diesel composition according to claim 1, wherein the substituted p-phenylene diamine of component (a) is one or more selected from the group consisting of di-substituted p-phenylene diamines with substituents having between 4 and 10 carbon atoms.

4. The diesel composition according to claim 3, wherein said substituted p-phenylene diamine is N-phenyl-N'-cyclohexyl-p-phenylene diamine, N,N-(1,3-dimethylbutyl)-N'-phenyl-p-phenylene diamine, N,N'-bis-(1,4-dimethylamyl)-p-phenylene diamine, N-p-tolyl-N'-(1,3-dimethylbutyl)-p-phenylene diamine, N,N'-diheptyl-p-phenylene diamine, N-isopropyl-N'-phenyl-p-phenylene diamine, N-isopropyl-N'-p-tolyl-p-phenylene diamine, N,N'-xylyl-p-phenylene diamine, N,N'-diphenyl-p-phenylene diamine, N,N'-di-(β-naphthyl)-p-phenylene diamine, N,N'-di-sec-butyl-p-phenylene diamine, N,N'-dioctyl-p-phenylene diamine, N,N'-bis-(1-methylheptyl) p-phenylene diamine, N,N'-bis-(1-ethyl-3-methylamyl) p-phenylene diamine, N,N'-bis-(1,4-dimethylbutyl) p-phenylene diamine, N-octyl-N'-phenyl-p-phenylene diamine, N-isobutyl-N'-phenyl-p-phenylene diamine, N,N'-dimethyl-N,N'-bis-(1-methylpropyl) p-phenylene diamine, N-(p-toluene sulfonyl)-N'-phenyl-p-phenylene diamine, N-(3-methylpropenylacryloxo-2-hydroxypropyl)-N'-phenyl-p-phenylene diamine, N-(3-anilinophenyl)methylacrylamide, or N-hexyl-N'-phenyl-p-phenylene diamine.

5. The diesel composition according to claim 3, wherein said substituted p-phenylene diamine is one or more of N,N-(1,3-dimethylbutyl)-N'-phenyl-p-phenylene diamine, N-octyl-N'-phenyl-p-phenylene diamine, N,N'-diheptyl-p-phenylene diamine, N,N'-di-sec-butyl-p-phenylene diamine, N,N'-bis-(1-ethyl-3-methylamyl) p-phenylene diamine, N,N'-bis-(1,4-dimethylbutyl) p-phenylene diamine, N,N'-dioctyl-p-phenylene diamine, and N,N'-bis-(1-methylheptyl) p-phenylene diamine.

6. The diesel composition according to claim 1, wherein the polyene polyamine of the structural formula H₂N[(CH₂)ₓ₂NH]_{y1}R₆ is one or more of ethylene diamine, diethylene triamine, triethylene tetramine, tetraethylene pentamine, pentaethylene hexamine, hexaethylene heptamine, heptaethylene octamine, propylene diamine, dipropylene triamine, tripropylene tetramine, tetrapropylene pentamine, pentapropylene hexamine, hexapropylene heptamine, heptapropylene octamine, and N,N'-bis(3-aminopropyl)-ethylene diamine, or one or more polyene polyamines wherein R₆ is n-butyl, n-amyl, n-hexyl, n-heptyl, n-octyl, n-nonyl, n-decyl, n-undecyl, n-dodecyl, n-tetradecyl, n-hexadecyl, n-octadecyl, n-eicosyl, n-didodecyl, iso-butyl, tert-butyl, iso-amyl, neo-amyl, iso-hexyl, iso-heptyl, iso-octyl, iso-nonyl, iso-decyl, iso-dodecyl, iso-tetradecyl, iso-hexadecyl, iso-octadecyl, iso-eicosyl, 9-octadecene, phenylmethyl, phenylethyl or phenylpropyl; a polyamine represented by the formula is a polyether diamine with the CAS number 9046-10-0 and having a Mn of 400; a polyamine represented by the formula (A2) is an imidazoline-type polyamine wherein y2 is an integer from 1 to 3, and R₇ is C₆-C₂₀ alkyl or C₆-C₂₀ alkenyl; said piperidine-type polyam-ine is 4-amino-2,2,6,6-tetramethylpiperidine or 1-(2-aminoethyl)piperidine; the tertiary amine containing polyamine of the formula (A4) is one or more of N,N-dimethyl-1,3-propylene diamine, N,N-diethyl-1,3-propylene diamine, N,N-dibutyl-1,3-propylene diamine, N,N-dimethyl-1,4-butylene diamine, N,N-diethyl-1,4-butylene diamine, N,N-dimethyl-1,6-hexanediamine; the tertiary amine containing polyamine of the formula (A5) is tri-(2-aminoethyl) amine; the tertiary amine containing polyamine of the formula (A6) is N,N-bis-(3-aminopropyl) methylamine.

7. The diesel composition according to claim 1 or 2, wherein said derivatives of polyamines are the reaction products of the ammonolysis reaction of one or more fatty acids having 6 to 40 carbon atoms, fatty acyl halides having 6 to 40 carbon atoms, or fatty acid alkyl esters having 6 to 40 carbon atoms with the above-mentioned polyamines, preferably wherein said fatty acid is one or more selected from the group consisting of caproic acid, adipic acid, octanoic acid, isooctanoic acid (2-ethylcaproic acid), capric acid, dodecanic acid, tetradecanoic acid, hexadecanoic acid (palmitic acid), octadecanoic acid (stearic acid), oleic acid, linoleic acid, linolenic acid, ricinolic acid, eicosenoic acid, arachidic acid, erucic acid, docosenoic acid, dimers of oleic acid and/or linoleic acid, industrial dimer acids, soybean oil acid, peanut oil acid, rapeseed oil acid, ricinoleic acid, and tall oil fatty acid; said fatty acyl halide is an acyl halide of the above-mentioned fatty acid; said fatty acid alkyl ester is a C1-C5 alkyl ester of the above-mentioned fatty acid, in particular biodiesel.

8. The diesel composition according claim 1 or 2, wherein conditions for said condensation reaction include a molar ratio of total polyamines to C1-C6 aldehyde of 1: (0.1-10), and a reaction temperature of 80-150 °C, wherein said C1-C6 aldehyde is one or more of formaldehyde, acetaldehyde, propionaldehyde, cyclo-caproaldehyde, and an aqueous solution of one or more of them.

9. The diesel composition according to claim 1, wherein said acylating agent is one or more of maleic acid, succinic acid, fumaric acid, itaconic acid, citraconic acid, isatoic acid, phthalic acid, maleic anhydride, succinic anhydride, itaconic anhydride, citraconic anhydride, isatoic anhydride and phthalic anhydride, and the half esters thereof, all of which are substituted by C6-C30 hydrocarbyl.

10. The diesel composition according to claim 1, wherein said acylating agent is one or more of C6-C30 hydrocarbyl substituted succinic acid, C6-C30 hydrocarbyl substituted succinic anhydride, and the half esters thereof.

11. The diesel composition according to claim 1, wherein said acylating agent is one or more of nonylsuccinic acid, decylsuccinic acid, dodecylsuccinic acid, tridecylsuccinic acid, tetradecylsuccinic acid, pentadecylsuccinic acid, hexadecylsuccinic acid, octadecylsuccinic acid, nonenylsuccinic acid, decenylsuccinic acid, dodecenylsuccinic acid, tetradecenylsuccinic acid, cetenylsuccinic acid, octadecenesuccinic acid, docosenylsuccinic acid, nonylsuccinic anhydride, decylsuccinic anhydride, dodecylsuccinic anhydride, tridecylsuccinic anhydride, tetradecylsuccinic anhydride, pentadecylsuccinic anhydride, hexadecylsuccinic anhydride, octadecylsuccinic anhydride, nonenylsuccinic anhydride, decenylsuccinic anhydride, dodecenylsuccinic anhydride, tetradecenylsuccinic anhydride, cetenylsuccinic anhydride, octadecenesuccinic anhydride, docosenylsuccinic anhydride, and the half esters thereof.

12. The diesel composition according to claim 1 or 2, wherein said diesel composition further comprises component (c), which is a metal deactivator capable of reacting with a metal surface and/or a metal chelator capable of reacting with or binding to a metal or metal ion.

13. The diesel composition according to claim 12, wherein the weight ratio of said component (a) to said component (c) is 1: 0.01-1.

14. The diesel composition according to claim 12, wherein said component (c) is one or more of benzotriazole, an ammonium salt formed by benzotriazole and a fatty amine, a product obtained by the Mannich reaction of benzotriazole, formaldehyde and a fatty amine, Schiff's base, and organic polycarboxylic acids, in particular wherein said Schiff's base may be N,N'-disalicylidene-1,2-propylene diamine; said organic polycarboxylic acid is tartaric acid.

15. The diesel composition according to claim 1 or 2, wherein said additive composition is present in an amount of 50-10000 ppm, relative to the amount of the base diesel.

16. The diesel composition according to claim 1 or 2, wherein said base diesel further comprises one or more additional diesels selected from the group consisting of petroleum diesel, Fischer-Tropsch synthetic diesel, hydrocracked biodiesel, and an oxygen-containing diesel concoction, wherein the ratio of the volume of said biodiesel to the volume of said additional diesels is 1: 0-99.

17. A method of increasing the oxidation stability of biodiesel, comprising adding, in a biodiesel-containing base diesel, an additive composition according to claim 1.

## Patentansprüche

1. Dieselzusammensetzung, die einen Basisdiesel und eine Additivzusammensetzung umfasst, **dadurch gekennzeichnet, dass** der Basisdiesel Biodiesel umfasst, und die Additivzusammensetzung Komponente (a) und Komponente (b) umfasst, wobei die Komponente (a) ein substituiertes p-Phenylendiamin ist und die Komponente (b) ein oder mehrere Polyamine oder Derivate davon ist, wobei das Polyamin ein Polyetherdiamin der Formel (A1):
wobei x1 eine ganze Zahl von 1 bis 10 ist, R₄ H oder ein Hydrocarbyl mit 1 bis 30 Kohlenstoffatomen ist, und R₅ H oder Methyl ist; oder
ein Polyenpolyamin der Strukturformel:
H₂N[(CH₂)ₓ₂NH]_{y1}R₆
wobei x2 eine ganze Zahl von 2 bis 4 ist, y1 eine ganze Zahl von 1 bis 8 ist, und R₆ H oder ein Hydrocarbyl mit 1 bis 30 Kohlenstoffatomen ist, und/oder ein Kondensat des Polyenpolyamins mit Ethylenoxid und/oder Propylenoxid; oder
ein Polyamin vom Imidazolin-Typ der Formel (A2):
wobei y2 eine ganze Zahl von 0 bis 5 ist, und R₇ ein Hydrocarbyl mit 1 bis 24 Kohlenstoffatomen ist; oder
ein Polyamin vom Piperazin-Typ, bei dem es sich um N-(2-Aminoethyl)piperazin oder N,N'-Di-(aminoethyl)piperazin handelt; oder
ein Polyamin vom Piperidin-Typ; oder
ein tertiäres Amin enthaltendes Polyamin der Formel (A4), (A5) oder (A6) ist:
wobei R₉ und R₁₀ Hydrocarbyle mit 1 bis 24 Kohlenstoffatomen sind, und x4 eine ganze Zahl von 0 bis 10 ist; oder
wobei x5 eine ganze Zahl von 1 bis 10 ist; oder
wobei R₁₁ ein Hydrocarbyl mit 1 bis 24 Kohlenstoffatomen ist, und x6 eine ganze Zahl von 1 bis 10 ist, und vorzugsweise eine ganze Zahl von 2 bis 6; wobei die Derivate der Polyamine die Reaktionsprodukte der Ammonolysereaktion von einer oder mehreren organischen Säuren mit 6 bis 40 Kohlenstoffatomen, Acylhalogeniden mit 6 bis 40 Kohlenstoffatomen oder organischen Säurealkylestern mit 6 bis 40 Kohlenstoffatomen mit den oben erwähnten Polyaminen sind, oder
wobei die Derivate der Polyamine die Reaktionsprodukte der Kondensationsreaktion der Polyamine mit C1-C6-Aldehyd sind, oder
wobei die Derivate der Polyamine die Reaktionsprodukte der Ammonolysereaktion eines Acylierungsmittels, das zwei Acylgruppen in einem Molekül enthält, mit den oben erwähnten Polyaminen in einem molaren Verhältnis von 1: (0,5-2) sind, wobei das Acylierungsmittel, das zwei Acylgruppen in einem Molekül enthält, eines oder mehrere einer C6-C30-Hydrocarbyl-substituierten organischen Dicarbonsäure, eines C6-C30-Hydrocarbyl-substituierten Anhydrids, und eines C6-C30-Hydrocarbyl-substituierten Halbesters ist; und wobei das Gewichtsverhältnis der Komponente (b) zu der Komponente (a) 0,01-100: 1 beträgt.

2. Dieselzusammensetzung gemäß Anspruch 1, wobei das Gewichtsverhältnis der Komponente (b) zu der Komponente (a) 0,05-10:1 beträgt.

3. Dieselzusammensetzung gemäß Anspruch 1, wobei das substituierte p-Phenylendiamin der Komponente (a) ein oder mehrere ausgewählt aus der Gruppe bestehend aus di-substituierten p-Phenylendiaminen mit Substituenten mit zwischen 4 und 10 Kohlenstoffatomen ist.

4. Dieselzusammensetzung gemäß Anspruch 3, wobei das substituierte p-Phenylendiamin N-Phenyl-N'-cyclohexyl-p-phenylendiamin, N,N-(1,3-Dimethylbutyl)-N'-phenyl-p-phenylendiamin, N,N'-Bis-(1,4-dimethylamyl)-p-phenylendiamin, N-p-Tolyl-N'-(1,3-dimethylbutyl)-p-phenylendiamin, N,N'-Diheptyl-p-phenylendiamin, N-Isopropyl-N'-phenyl-p-phenylendiamin, N-Isopropyl-N'-p-tolyl-p-phenylendiamin, N,N'-Xylyl-p-phenylendiamin, N,N'-Diphenyl-p-phenylendiamin, N,N'-Di-(β-naphthyl)-p-phenylendiamin, N,N'-Di-sec-butyl-p-phenylendiamin, N,N'-Dioctyl-p-phenylendiamin, N,N'-Bis-(1-methylheptyl)-p-phenylendiamin, N,N-Bis-(1-ethyl-3-methylamyl)-p-phenylendiamin, N,N'-Bis-(1,4-dimethylbutyl)-p-phenylendiamin, N-Octyl-N'-phenyl-p-phenylendiamin, N-Isobutyl-N'-phenyl-p-phenylendiamin, N,N'-Dimethyl-N,N'-bis-(1-methylpropyl)-p-phenylendiamin, N-(p-Toluolsulfonyl)-N'-phenyl-p-phenylendiamin, N-(3-Methylpropenylacryloxo-2-hydroxypropyl)-N'-phenyl-p-phenylendiamin, N-(3-Anilinophenyl)methylacrylamid oder N-Hexyl-N'-phenyl-p-phenylendiamin ist.

5. Dieselzusammensetzung gemäß Anspruch 3, wobei das substituierte p-Phenylendiamin ein oder mehrere von N,N-(1,3-Dimethylbutyl)-N'-phenyl-p-phenylendiamin, N-Octyl-N'-phenyl-p-phenylendiamin, N,N'-Diheptyl-p-phenylendiamin, N,N'-Di-sec-butyl-p-phenylendiamin, N,N-Bis-(1-ethyl-3-methylamyl)-p-phenylendiamin, N,N'-Bis-(1,4-dimethylbutyl)-p-phenylendiamin, N,N'-Dioctyl-p-phenylendiamin und N,N'-Bis-(1-methylheptyl)-p-phenylendiamin ist.

6. Dieselzusammensetzung gemäß Anspruch 1, wobei das Polyenpolyamin der Strukturformel H₂N[(CH₂)ₓ₂NH]_{y1}R₆ eines oder mehrere ist von Ethylendiamin, Diethylentriamin, Triethylentetramin, Tetraethylenpentamin, Pentaethylenhexamin, Hexaethylenheptamin, Heptaethylenoctamin, Propylendiamin, Dipropylentriamin, Tripropylentetramin, Tetrapropylenpentamin, Pentapropylenhexamin, Hexapropylenheptamin, Heptapropylenoctamin und N,N'-Bis-(3-aminopropyl)-ethylendiamin, oder ein oder mehrere Polyenpolyamine, wobei R₆ Butyl, n-Amyl, n-Hexyl, n-Heptyl, n-Octyl, n-Nonyl, n-Decyl, n-Undecyl, n-Dodecyl, N-Tetradecyl, n-Hexadecyl, n-Octadecyl, n-Eicosyl, n-Didodecyl, iso-Butyl, tert-Butyl, iso-Amyl, neo-Amyl, iso-Hexyl, iso-Heptyl, iso-Octyl, iso-Nonyl, iso-Decyl, iso-Dodecyl, iso-Tetradecyl, iso-Hexadecyl, iso-Octadecyl, iso-Eicocyl, 9-Octadecen, Phenylmethyl, Phenylethyl oder Phenylpropyl ist; ein durch die Formel dargestelltes Polyamin ein Polyetherdiamin mit derCAS-Nummer 9046-10-0 und mit einem Mn von 400 ist; ein durch die Formel (A2) dargestelltes Polyamin ein Polyamin vom Imidazolin-Typ ist, wobei y2 eine ganze Zahl von 1 bis 3 ist und R₇ C₆-C₂₀-Alkyl oder C₆-C₂₀-Alkenyl ist; das Polyamin vom Piperidin-Typ 4-Amino-2,2,6,6-tetramethylpiperidin oder 1-(2-Aminoethyl)piperidin ist; das ein tertiäres Amin enthaltende Polyamin der Formel (A4) ein oder mehrere von N,N-Dimethyl-1,3-propylendiamin, N,N-Diethyl-1,3-propylendiamin, N,N-Dibutyl-1,3-propylendiamin, N,N-Dimethyl-1,4-butylendiamin, N,N-Diethyl-1,4-butylendiamin, N,N-Dimethyl-1,6-hexandiamin ist; das ein tertiäres Amin enthaltende Polyamin der Formel (A5) Tri-(2-aminoethyl)amin ist; das ein tertiäres Amin enthaltende Polyamin der Formel (A6) N,N-Bis-(3-aminopropyl)methylamin ist.

7. Dieselzusammensetzung gemäß Anspruch 1 oder 2, wobei die Derivate der Polyamine die Reaktionsprodukte der Ammonolysereaktion von einer oder mehreren Fettsäuren mit 6 bis 40 Kohlenstoffatomen, Fettacylhalogeniden mit 6 bis 40 Kohlenstoffatomen oder Fettsäurealkylestern mit 6 bis 40 Kohlenstoffatomen mit den oben erwähnten Polyaminen sind, vorzugsweise wobei die Fettsäure eine oder mehrere ist ausgewählt aus der Gruppe bestehend aus Capronsäure, Adipinsäure, Octansäure, Isooctansäure (2-Ethylcapronsäure), Caprinsäure, Dodecansäure, Tetradecansäure, Hexadecansäure (Palmitinsäure), Octadecansäure (Stearinsäure), Ölsäure, Linolsäure, Linolensäure, Ricinolsäure, Eicosensäure, Arachinsäure, Erucasäure, Docosensäure, Dimere von Ölsäure und/oder Linolensäure, industrielle Dimersäuren, Sojabohnenölsäure, Erdnussölsäure, Rapsölsäure, Ricinolsäure und Tallölfettsäure; das Fettacylhalogenid ein Acylhalogenid der oben erwähnten Fettsäure ist; der Fettsäurealkylester ein C1-C5 Alkylester der oben erwähnten Fettsäure ist, insbesondere Biodiesel.

8. Dieselzusammensetzung gemäß Anspruch 1 oder 2, wobei die Bedingungen für die Kondensationsreaktion ein molares Verhältnis von Gesamtpolyaminen zu C1-C6-Aldehyd von 1: (0,1-10) und eine Reaktionstemperatur von 80-150°C einschließen, wobei das C1-C6-Aldehyd ein oder mehrere von Formaldehyd, Acetaldehyd, Propionaldehyd, Cyclocaproaldehyd und einer wässrigen Lösung von einem oder mehreren davon ist.

9. Dieselzusammensetzung gemäß Anspruch 1, wobei das Acylierungsmittel eines oder mehrere ist von Maleinsäure, Bernsteinsäure, Fumarsäure, Itaconsäure, Citraconsäure, Isatinsäure, Phthalsäure, Maleinsäureanhydrid, Bernsteinsäureanhydrid, Itaconsäureanhydrid, Citraconsäureanhydrid, Isatinsäureanhydrid und Phthalsäureanhydrid und den Halbestern davon, von denen alle durch C6-C30-Hydrocarbyl substituiert sind.

10. Dieselzusammensetzung gemäß Anspruch 1, wobei das Acylierungsmittel eines oder mehrere ist von C6-C30-Hydrocarbyl-substituierter Bernsteinsäure, C6-C30-Hydrocarbyl-substituiertem Bernsteinsäureanhydrid und den Halbestern davon.

11. Dieselzusammensetzung gemäß Anspruch 1, wobei das Acylierungsmittel eines oder mehrere ist von Nonylbernsteinsäure, Decylbernsteinsäure, Dodecylbernsteinsäure, Tridecylbernsteinsäure, Tetradecylbernsteinsäure, Pentadecylbernsteinsäure, Hexadecylbernsteinsäure, Octadecylbernsteinsäure, Nonenylbernsteinsäure, Decenylbernsteinsäure, Dodecenylbernsteinsäure, Tetradecenylbernsteinsäure, Cetenylbernsteinsäure, Octadecenbernsteinsäure, Docosenylbernsteinsäure, Nonylbernsteinsäureandhydrid, Decylbernsteinsäureanhydrid, Dodecylbernsteinsäureanhydrid, Tridecylbernsteinsäureanhydrid, Tetradecylbernsteinsäureanhydrid, Pentaldecylbernsteinsäureanhydrid, Hexadecylbernsteinsäureanhydrid, Octadecylbernsteinsäureanhydrid, Nonenylbernsteinsäureanhydrid, Decenylbernsteinsäureanhydrid, Dodecenylbernsteinsäureanhydrid, Tetradecenylbernsäureanhydrid, Cetenylbernsteinsäureanhydrid, Octadecenbernsteinsäureanhydrid, Docosenylbernsteinsäureanhydrid, und den Halbestern davon.

12. Dieselzusammensetzung gemäß Anspruch 1 oder 2, wobei die Dieselzusammensetzung weiterhin Komponente (c) umfasst, bei der es sich um einen Metalldeaktivator, der zur Reaktion mit einer Metalloberfläche befähigt ist, und/oder einen Metallchelator, der zur Reaktion mit einem Metall oder Metallion oder zur Bindung an ein Metall oder Metallion befähigt ist, handelt.

13. Dieselzusammensetzung gemäß Anspruch 12, wobei das Gewichtsverhältnis der Komponente (a) zu der Komponente (c) 1:0,01-1 beträgt.

14. Dieselzusammensetzung gemäß Anspruch 12, wobei die Komponente (c) eines oder mehrere ist von Benzotriazol, einem aus Benzotriazol und einem Fettamin gebildeten Ammoniumsalz, einem durch die Mannich-Reaktion von Benzotriazol, Formaldehyd und einem Fettamin erhaltenen Produkt, Schiff sehe Base, und organischen Polycarbonsäuren, insbesondere wobei die Schiff sehe Base N,N'-Disalicyliden-1,2-propylendiamin sein kann; die organische Polycarbonsäure Weinsäure ist.

15. Dieselzusammensetzung gemäß Anspruch 1 oder 2, wobei die Additivzusammensetzung in einer Menge von 50-10000 ppm, relativ zu der Menge des Basisdiesels, vorliegt.

16. Dieselzusammensetzung gemäß Anspruch 1 oder 2, wobei der Basisdiesel weiterhin ein oder mehrere zusätzliche Diesel umfasst, ausgewählt aus der Gruppe bestehend aus Erdöldiesel, Fischer-Tropsch-Synthetikdiesel, hydrogecracktem Biodiesel, und einem sauerstoffhaltigen Gebräu, wobei das Verhältnis des Volumens des Biodiesels zu dem Volumen des zusätzlichen Diesels 1:0-99 beträgt.

17. Verfahren zur Erhöhung der Oxidationsstabilität von Biodiesel, umfassend das Hinzufügen einer Additivzusammensetzung gemäß Anspruch 1 in einen Biodiesel enthaltenden Basisdiesel.

## Revendications

1. Composition de diesel, qui comprend un diesel de base et une composition additive, **caractérisée en ce que** ledit diesel de base comprend un biodiesel, et ladite composition additive comprend un composant (a) et un composant (b), ledit composant (a) étant une p-phénylènediamine substituée, et ledit composant (b) étant une ou plusieurs polyamines ou un ou plusieurs dérivés de celles-ci, la polyamine étant une polyétherdiamine de formule (A1)
dans laquelle x1 est un entier de 1 à 10, R₄ est H ou un groupe hydrocarbyle ayant 1 à 30 atomes de carbone, et R₅ est H ou le groupe méthyle ; ou une polyènepolyamine de de formule développée :
H₂N[(CH₂)ₓ₂NH]_{y1}R₆
dans laquelle x2 est un entier de 2 à 4, y1 et un entier e 1 à 8, et R₆ est H ou un groupe hydrocarbyle ayant 1 à 30 atomes de carbone, et/ou un produit de condensation de ladite polyènepolyamine avec de l'oxyde d'éthylène et/ou de l'oxyde de propylène ; ou
une polyamine de type imidazoline de formule (A2) ;
dans laquelle y2 est un entier de 0 à 5, et R₇ est un groupe hydrocarbyle ayant 1 à 24 atomes de carbone ; ou une polyamine de type pipérazine, qui est la N-(2-aminoéthyl)pipérazine ou la N,N'-di(aminoéthyl)-pipérazine ; ou
une polyamine de type pipéridine ; ou
une amine tertiaire contenant une polyamine de formule (A4), (A5) ou (A6) :
dans laquelle R₉ et R₁₀ sont des groupes hydrocarbyle ayant 1 à 24 atomes de carbone, et x4 est un entier de 0 à 10 ; ou
dans laquelle x5 est un entier de 1 à 10 ; ou
dans laquelle R₁₁ est un groupe hydrocarbyle ayant 1 à 24 atomes de carbone, et x6 est un entier de 1 à 10, de préférence un entier de 2 à 6 ;
dans laquelle lesdits dérivés de polyamines sont les produits de réaction de la réaction d'ammonolyse d'un ou plusieurs acides organiques ayant 6 à 40 atomes de carbone, halogénures d'acyle ayant 6 à 40 atomes de carbone, ou esters alkyliques d'acides organiques ayant 6 à 40 atomes de carbone, avec les polyamines mentionnées ci-dessus, ou
dans laquelle lesdits dérivés de polyamines sont les produits de réaction de la réaction de condensation desdites polyamines avec un aldéhyde en C₁-C₆, ou
dans laquelle lesdits dérivés de polyamines sont les produits de réaction de la réaction d'ammonolyse d'un agent d'acylation contenant deux groupes acyle par molécule avec les polyamines mentionnées ci-dessus selon un rapport en moles de 1:(0,5-2), ledit agent d'acylation contenant deux groupes acyle par molécule étant un ou plusieurs acides dicarboxyliques organiques à substitution hydrocarbyle en C₆-C₃₀, un anhydride à substitution hydrocarbyle en C₆-C₃₀, un semi-ester à substitution hydrocarbyle en C₆-C₃₀ ;
et le rapport en poids dudit composant (b) audit composant (a) étant de 0,01 à 100:1.

2. Composition de diesel selon la revendication 1, dans laquelle le rapport en poids dudit composant (b) audit composant (a) est de 0,05 à 10:1.

3. Composition de diesel selon la revendication 1, dans laquelle la p-phénylènediamine substituée du composant (a) est une ou plusieurs choisies dans le groupe consistant en les p-phénylènediamines disubstituées par des substituants ayant de 4 à 10 atomes de carbone.

4. Composition de diesel selon la revendication 3, dans laquelle ladite p-phénylènediamine substituée est la N-phényl-N'-cyclohexyl-p-phénylènediamine, la N,N-(1,3-diméthylbutyl)-N'-phényl-p-phénylènediamine, la N,N'-bis(1,4-diméthylamyl)-p-phénylènediamine, la N-p-tolyl-N'-(1,3-diéthylbutyl)-p-phénylènediamine, la N,N'-diheptyl-p-phénylènediamine, la N-isopropyl-N'-phényl-p-phénylènediamine, la N-isopropyl-N'-p-tolyl-p-phénylènediamine, la N,N'-xylyl-p-phénylènediamine, la N,N'-diphényl-p-phénylènediamine, la N,N'-di(β-naphtyl)-p-phénylènediamine, la N,N'-di-sec-butyl-p-phénylènediamine, la N,N'-dioctyl-p-phénylènediamine, la N,N'-bis(1-méthylheptyl)-p-phénylènediamine, la N,N'-bis(1-éthyl-3-méthylamyl)-p-phénylènediamine, la N,N'-bis(1,4-diméthylbutyl)-p-phénylènediamine, la N-octyl-N'-phényl-p-phénylènediamine, la N-isobutyl-N'-phényl-p-phénylènediamine, la N,N'-diméthyl-N,N'-bis(1-méthylpropyl)-p-phénylènediamine, la N-p-toluènesulfonyl)-N'-phényl-p-phénylènediamine, la N-(3-méthylpropénylacryloxo-2-hydroxypropyl)-N'-phényl-p-phénylènediamine, le N-(3-anilinophényl)-méthylacrylamide ou la N-hexyl-N'-phényl-p-phénylènediamine.

5. Composition de diesel selon la revendication 3, dans laquelle ladite p-phénylènediamine substituée est une ou plusieurs de la N,N'-(1,3-diméthylbutyl)-N'-phényl-p-phénylènediamine, de la N-octyl-N'-phényl-p-phénylènediamine, de la N,N'-diheptyl-p-phénylènediamine, de la N,N'-di-sec-butyl-p-phénylènediamine, de la N,N'-bis(1-éthyl-3-méthylamyl)-p-phénylènediamine, de la N,N'-bis(1,4-diméthylbutyl)-p-phénylènediamine, de la N,N'-dioctyl-p-phénylènediamine et de la N,N'-bis(1-méthylheptyl)-p-phénylènediamine.

6. Composition de diesel selon la revendication 1, dans laquelle la polyènepolyamine de formule développée H₂N[(CH₂)ₓ₂NH]_{y1}R₆ est une ou plusieurs de l'éthylènediamine, de la diéthylènetriamine, de la triéthylènetétramine, de la tétraéthylènepentamine, de la pentaéthylène-hexamine, de l'hexaéthylène-heptamine, de l'heptaéthylène-octamine, de la propylènediamine, de la dipropylènetriamine, de la tripropylènetétramine, de la tétrapropylènepentamine, de la pentapropylène-hexamine, de l'hexapropylène-heptamine, de l'heptapropylène-octamine et de la N,N'-bis(3-aminopropyl)-éthylènediamine, ou une ou plusieurs polyènediamines dans lesquelles R₆ est le groupe n-butyle, n-amyle, n-hexyle, n-heptyle, n-octyle, n-nonyle, n-décyle, n-undécyle, n-dodécyle, n-tétradécyle, n-hexadécyle, n-octadécyle, n-éicosyle, n-didodécyle, isobutyle, tert-butyle, isoamyle, néoamyle, isohexyle, isoheptyle, isooctyle, isononyle, isodécyle, isododécyle, isotétradécyle, isohexadécyle, isooctadécyle, isoéicosyle, 9-octadécène, phénylméthyle, phényléthyle ou phénylpropyle ; une polyamine représentée par la formule est une polyétherdiamine ayant le numéro CAS 9046-10-0 et ayant une Mn de 400 ; une polyamine représentée par la formule (A2) est une polyamine de type imidazoline dans laquelle y2 est un entier de 1 à 3, et R₇ est un groupe alkyle en C₆-C₂₀ ou alcényle en C₆-C₂₀ ; ladite polyamine de type pipéridine est la 4-amino-2,2,6,6-tétramétylpipéridine ou la 1-(2-aminoéthyl)pipéridine ; la polyamine de formule (A4) contenant une amine tertiaire est une ou plusieurs de la N,N-diméthyl-1,3-propylènediamine, de la N,N-diéthyl-1,3-propylènediamine, de la N,N-dibutyl-1,3-propylènediamine, de la N,N-diméthyl-1,4-butylènediamine, de la N,N-diéthyl-1,4-butylènediamine, de la N,N-diméthyl-1,6-hexanediamine ; la polyamine contenant une amine tertiaire de formule (A5) est la tri(2-aminoéthyl)amine ; la polyamine contenant une amine tertiaire de formule (A6) est la N,N'-bis(3-aminopropyl)-méthylamine.

7. Composition de diesel selon la revendication 1 ou 2, dans laquelle lesdits dérivés de polyamines sont les produits de réaction de la réaction d'ammonolyse d'un ou plusieurs acides gras ayant 6 à 40 atomes de carbone, halogénures d'acyle gras ayant 6 à 40 atomes de carbone ou esters alkyliques d'acides gras ayant 6 à 40 atomes de carbone avec les polyamines mentionnées ci-dessus, de préférence dans laquelle ledit acide gras est un ou plusieurs choisis dans le groupe consistant en l'acide caproïque, l'acide adipique, l'acide octanoïque, l'acide isooctanoïque (acide 2-éthylcaproïque), l'acide caprique, l'acide dodécanoïque, l'acide tétradécanoïque, l'acide hexadécanoïque (acide palmitique), l'acide octadécanoïque (acide stéarique), l'acide oléique, l'acide linoléique, l'acide linolénique, l'acide ricinoléique, l'acide éicosénoïque, l'acide arachidique, l'acide érucique, l'acide docosénoïque, les dimères de l'acide oléique et/ou de l'acide linoléique, les acides dimères industriels, l'acide dérivé de l'huile de soja, l'acide dérivé de l'huile d'arachide, l'acide dérivé de l'huile de colza, l'acide ricinoléique, l'acide gras dérivé du tallol ; ledit halogénure d'acyle gras est un halogénure d'acyle de l'acide gras mentionné ci-dessus ; ledit ester alkylique d'acide gras est un ester alkylique en C₁-C₅ de l'acide gras mentionné ci-dessus, en particulier le biodiesel.

8. Composition de diesel selon la revendication 1 ou 2, dans laquelle les conditions de ladite réaction de condensation comprennent un rapport en moles des polyamines totales à l'aldéhyde en C₁-C₆ de 1:(0,1-10), et une température de réaction de 80 à 150 °C, ledit aldéhyde en C₁-C₆ étant un ou plusieurs du formaldéhyde, de l'acétaldéhyde, du propionaldéhyde, du cyclo-caproaldéhyde, et une solution aqueuse d'un ou plusieurs d'entre eux.

9. Composition de diesel selon la revendication 1, dans laquelle ledit agent d'acylation est un ou plusieurs de l'acide maléique, de l'acide succinique, de l'acide fumarique, de l'acide itaconique, de l'acide citraconique, de l'acide isatoïque, de l'acide phtalique, de l'anhydride maléique, de l'anhydride succinique, de l'anhydride itaconique, de l'anhydride citraconique, de l'anhydride isatoïque et de l'anhydride phtalique, et les semi-esters de ceux-ci, dont tous sont substitués par un groupe hydrocarbyle en C₆-C₃₀.

10. Composition de diesel selon la revendication 1, dans laquelle ledit agent d'acylation est un ou plusieurs de l'acide succinique à substitution hydrocarbyle en C₆-C₃₀, de l'anhydride succinique à substitution hydrocarbyle en C₆-C₃₀, et des semi-esters de ceux-ci.

11. Composition de diesel selon la revendication 1, dans laquelle ledit agent d'acylation est un ou plusieurs de l'acide nonylsuccinique, de l'acide décylsuccinique, de l'acide dodécylsuccinique, de l'acide tridécylsuccinique, de l'acide tétradécylsuccinique, de l'acide pentadécylsuccinique, de l'acide hexadécylsuccinique, de l'acide octadécylsuccinique, de l'acide nonénylsuccinique, de l'acide décénylsuccinique, de l'acide dodécénylsuccinique, de l'acide tétradécénylsuccinique, de l'acide céténylsuccinique, de l'acide octadécènesuccinique, de l'acide docosénylsuccinique, de l'anhydride nonylsuccinique, de l'anhydride décylsuccinique, de l'anhydride dodécylsuccinique, de l'anhydride tridécylsuccinique, de l'anhydride tétradécylsuccinique, de l'anhydride pentadécylsuccinique, de l'anhydride hexadécylsuccinique, de l'anhydride octadécylsuccinique, de l'anhydride nonénylsuccinique, de l'anhydride décénylsuccinique, de l'anhydride dodécénylsuccinique, de l'anhydride tétradécylsuccinique, de l'anhydride céténylsuccinique, de l'anhydride octadécènesuccinique, de l'anhydride docosénylsuccinique, et des semi-esters de ceux-ci.

12. Composition de diesel selon la revendication 1 ou 2, dans laquelle ladite composition de diesel comprend un composant (c), qui est un désactivateur de métaux susceptible de réagir avec une surface métallique et/ou un chélatant de métaux susceptible de réagir avec un métal ou un ion métallique ou de se lier à celui-ci.

13. Composition de diesel selon la revendication 12, dans laquelle le rapport en poids dudit composant (a) audit composant (c) est de 1:0,01-1.

14. Composition de diesel selon la revendication 12, dans laquelle ledit composant (c) est un ou plusieurs du benzotriazole, d'un sel d'ammonium formé par le benzotriazole et une amine grasse, d'un produit obtenu par la réaction de Mannich du benzotriazole, du formaldéhyde et d'un acide gras, d'une base de Schiff et d'acides carboxyliques organiques, en particulier dans laquelle ladite base de Schiff peut être la N,N'-disalicylidène-1,2-propylènediamine ; ledit acide polycarboxylique organique étant l'acide tartrique.

15. Composition de diesel selon la revendication 1 ou 2, dans laquelle ladite composition additive est présente en une quantité de 50 à 10 000 ppm, par rapport à la quantité du diesel de base.

16. Composition de diesel selon la revendication 1 ou 2, dans laquelle ledit diesel de base comprend en outre un ou plusieurs diesels additionnels choisis dans le groupe consistant en le diesel de pétrole, le diesel synthétique de Fischer-Tropsch, le biodiesel hydrocraqué et une concoction de diesels oxygénés, le rapport en volume dudit biodiesel au volume desdits diesels additionnels étant de 1:0-99.

17. Procédé pour augmenter la stabilité à l'oxydation d'un biodiesel, comprenant l'addition, à un diesel de base contenant un biodiesel, d'une composition additive selon la revendication 1.
